

# United States Patent Office

3,113,026  
Patented Dec. 3, 1963

1

3,113,026

## POLYVINYL ALCOHOL PHOTOGRAPHIC SILVER HALIDE EMULSIONS

Joseph A. Sprung, Binghamton, N.Y., assignor to General Aniline & Film Corporation, New York, N.Y., a corporation of Delaware  
No Drawing. Filed Jan. 19, 1959, Ser. No. 787,363  
23 Claims. (Cl. 96—107)

This invention relates to photographic silver halide emulsions which comprise a silver halide dispersed in a polyvinyl alcohol polymer carrier and to photographic layers produced therefrom. More particularly, it relates to the control of the photographic properties of such silver halide polyvinyl alcohol emulsions by the use of various surface-active agents designated hereafter as photographic activators or sensitizers.

It has long been the goal of the photographic industry to replace gelatin with a more satisfactory carrying vehicle for the light-sensitive silver halide salts in photographic emulsions. Perhaps the main objection to the use of gelatin can be attributed to the fact that it is a natural product and, therefore, is subject to variations in composition which may cause difficulties in controlling the photographic properties of the emulsions prepared therefrom. For instance, each batch of fresh gelatin must ordinarily be submitted to a wide variety of tests, including the preparation of sample emulsions, to determine its photographic activity before it can be accepted for manufacturing use. In addition, photographic emulsions based on gelatin are brittle, subject to attack by bacteria and fungi and cannot be processed at elevated temperatures without special prior treatment. Despite the serious drawbacks, gelatin still remains the standard silver halide carrier in practically all commercial photographic emulsions. Its general acceptance, notwithstanding its many disadvantages, stems from the fact that it possesses a number of unique physical and chemical properties which make it ideal for photographic applications.

Gelatin is a thermo-reversible substance, and because of this property, the production of photographic emulsions prepared therefrom is greatly facilitated. The emulsions can be chilled to produce solid gels which can be subsequently shredded into particles and readily washed free of unwanted soluble salts by simple washing procedures. The thermo-reversibility of gelatin is also highly instrumental in facilitating the coating operation of photographic emulsions since setting of the liquid emulsion occurs immediately on contact with a chilled base.

Gelatin also functions as a peptizing agent for the insoluble silver salts, and provides the essential sensitizing and restraining principles which govern the light-sensitive characteristics of the silver halide grains.

The light-sensitivity of a gelatin silver halide photographic emulsion is determined mainly by: (1) the size and distribution of the silver halide grains and (2) the acquisition from the gelatin of certain sulfur chemical sensitizing constituents. The crystal growth in an emulsion is usually referred to as physical or Ostwald ripening, while the action of the sulfur sensitizers on the grains is known as chemical sensitization. By properly controlling the size and distribution and the chemical sensitization of the silver halide grains, photographic emulsions, having a wide variety of characteristics and applications, can be produced.

Various synthetic materials have been proposed as substitutes for gelatin but none, except possibly polyvinyl alcohol, has shown much promise as being able to satisfy the exacting photographic requirements.

Some of the desirable physical properties of polyvinyl alcohol which qualify it as a carrier for the silver halide salts in photographic emulsions are: (1) it is capable of

2

suspending silver halide grains; (2) the polyvinyl alcohol emulsions can be washed by dialysis, or can be precipitated and washed by decantation to remove the soluble salts; (3) the emulsions can be coated on paper or a suitable subbed film base; and (4) the coated emulsions can be hardened and processed in the conventional developing and fixing solutions.

While polyvinyl alcohol is acceptable mechanically as a silver halide carrying vehicle, it, nevertheless, lacks some of the physical and chemical features of gelatin which facilitate the preparation of photographic emulsions, particularly those in the high speed range. Pure polyvinyl alcohol, unlike gelatin, is highly restraining and does not permit the growth (Ostwald ripening) of the silver halide grains. In addition, unmodified polyvinyl alcohol silver halide emulsions cannot be ripened chemically to increased light-sensitivity with the conventional labile sulfur compounds known to be effective in the gelatin emulsion system. Since emulsion speed is dependent upon the attainment of proper grain size and response to chemical sensitization, it is apparent why polyvinyl alcohol has been used in the past only for the preparation of low speed contact printing papers.

It has now been discovered that the photographic properties of non-gelatin silver halide emulsions can be regulated or controlled by adjusting the surface charge on the silver halide grains by means of selected surface-active agents. The method of preparing such photographic emulsions constitutes an important object of this invention.

It is a further object of this invention to provide a polyvinyl alcohol silver halide photographic emulsion having surface-active agents incorporated therein to render it capable of grain growth (physical ripening) and chemical sensitization in the manner of the conventional gelatin emulsions.

It is a further object of this invention to provide a method for increasing the silver halide carrying capacity of polyvinyl alcohol.

It is a further object of this invention to provide polyvinyl alcohol silver halide emulsions which will respond to optical sensitization in the manner of the conventional gelatin emulsions.

A still further object is to provide a process of preparing polyvinyl alcohol silver halide photographic emulsions and emulsion layers therefrom which are equal in light-sensitivity to commercially available photographic materials.

Other objects will appear hereinafter as the description proceeds.

According to the present invention, polyvinyl alcohol silver halide emulsions of predetermined and predictable photographic characteristics can be produced by controlling the electrical charge pattern on the surface of the silver halide grains. Such a charge pattern is established by surrounding the light-sensitive grains with certain surface-active materials or activators which are adsorbed on the silver halide crystal surface. I have found that the desired electrical charge pattern can be achieved by preparing polyvinyl alcohol photographic emulsions in the presence of various surface-active amphotolytic or combinations of surface-active amphotolytic and cationic agents.

The surface-active substances which are useful for this invention are characterized by possessing an aliphatic chain of at least 8 carbon atoms which is linked to an anionic and/or cationic functional group. In the case of the cationic surface-active agents, the functional group may be represented by primary amino ( $-\text{NH}_2$ ), secondary amino ( $>\text{NH}$ ), tertiary amino

70



## quaternary ammonium

hydrazino ( $-\text{NH}-\text{NH}_2$ ), azonium

guanyl



guanido



biguanido



amine oxide



ternary sulfonium



or quaternary phosphonium



substituents.

Such surface-active cationic agents impart a positive charge on the silver halide grain surface to which they become adsorbed. By appropriate modifications in the chemical make-up of the cationic agents, the intensity of the positive charge can be varied. Since the photographic activity of the light-sensitive grains is closely associated with the nature of the positive charge, the structure of the cationics can be altered to produce silver halide emulsions having a variety of photographic properties.

However, silver halide emulsions sensitized with surface-active cationics tend to be foggy, a condition that calls for rather large quantities of stabilizers. As a consequence, the emulsions are slow and useful only for such limited applications as printing paper.

I have now found that the introduction of certain negative or acidic substituents into the cationic molecule gives rise to a sensitizing agent having greatly improved photographic properties compared to the unmodified cationic structure. The resulting entities, since they are characterized by residual positive and negative charges, are amphoteric in nature.

Typical of the acidic or negative substituents, which can be employed as modifiers in the manner described above, include: carboxylic acid ( $-\text{COOH}$ ), sulfonic acid ( $-\text{SO}_3\text{H}$ ), sulfenic acid ( $-\text{SO}_2\text{H}$ ), sulfuric ester

phosphonic acid ( $-\text{PO}_3\text{H}_2$ ), phosphonous acidphosphoric monoester ( $-\text{OPO}_3\text{H}_2$ ), phosphoric diestermercapto ( $-\text{SH}$ ), or phenolic hydroxy ( $-\text{OH}$ ) groups.

Since these amphoteric substances, sometimes referred to herein as ampholytes, contain both cationic and anionic substituents, they may be represented by the inner salt or "zwitterion" formula or they may be written as acid, basic or neutral salts. The particular form assumed by the ampholytes depends on their mode of preparation and on the pH of the surrounding medium.

The various forms may be represented as follows:



wherein  $\text{F}^+$  represents an onium grouping,  $\text{An}$  represents an acidic substituent of the type above,  $\text{Q}$  represents a divalent organic grouping containing an aliphatic chain of at least 8 carbon atoms,  $\text{X}^-$  represents an anion,  $\text{M}$  represents ammonium or an alkali metal, and  $\text{H}$  is hydrogen.

While many compounds embraced by the above formulae are suitable for my purpose, I normally employ those of the following formulae:



wherein  $\text{F}^+$  represents an ammonium group,  $\text{Q}$  represents a divalent organic grouping such as a chain comprising carbon, nitrogen, oxygen, sulfur or aryl rings of the benzene and naphthalene series,  $\text{X}^-$  represents an anion,  $\text{M}$  represents ammonium or alkali metal, and  $\text{H}$  is hydrogen.

Compounds falling within the ambit of the Formula I include aminocarboxylic acids, betaines, taurines and thetaines, said compounds having an aliphatic chain of at least 8 carbon atoms.

Illustrative of the surface-active materials of the type described above are compounds represented by the following formulae:

## CATIONICS



wherein  $\text{Alk}$  represents an aliphatic chain of at least 8 carbon atoms and  $\text{B}$  represents hydrogen, carboxeralkyl, carboxamido or amino groups.



wherein  $\text{Alk}$  has the value given above and  $\text{R}_1$  represents a lower alkyl group.



wherein  $\text{R}_2$  and  $\text{R}_3$  represent lower alkyl groups or together can form a heterocyclic ring system of the pyrrolidine series, piperidine series, pyridine series, morpholine series or quinoline series,  $\text{Alk}$  has the value given above and can be substituted by an amino group and  $\text{F}$  represents an intermediate linkage such as a carbon atom or

grouping such as  $-\text{NH---CO}(\text{CH}_2)_n-$  wherein  $n$  is an integer of from 1 to 4;  $-\text{NH---S---NH---CO}(\text{CH}_2)_n-$  wherein  $\text{S}$  can be a lower alkylaryl bridge of the benzene and naphthalene series and  $n$  has the value given above;

$-\text{CONH---}(\text{CH}_2)_n-$  wherein  $n$  has the value given above;  $-\text{Aryl---OCH}_2\text{CH}_2(\text{OCH}_2\text{CH}_2)_{m-1}-$  wherein  $m$  is an integer of from 1 to 3 and  $\text{Aryl}$  is an aryl group of the benzene and naphthalene series.



wherein  $\text{Alk}$  has the value given above and  $\text{R}_4$  is a heterocyclic ring system such as pyridine, quinoline and benzothiazole and the quaternary salts thereof.



wherein  $\text{Alk}$  has the values given above and  $\text{X}$  is an anion such as halogen, p-toluenesulfonate, chloride, etc., and  $\text{Y}$  can be hydrogen or  $-\text{O-Aryl-}$  wherein  $\text{Aryl}$  is a mono or bicyclic aromatic radical.



and



wherein Alk, X and Y have the values given above.



wherein  $R_1$  and Alk have the value given above;  $R_4$  represents lower alkyl which can be substituted by aryl groups of the benzene and naphthalene series, carbamyl groups, lower alkoxy carbonyl groups, 2-succimidyl groups, lower alkylamido groups, acyl groups and heterocyclic nuclei of the pyridine, quinoline and benzothiazole series; U represents a single carbon-nitrogen linkage, a bridge such as  $-\text{Aryl}-\text{OCH}_2-\text{SH}_2-(\text{OCH}_2-\text{CH}_2)_{m-1}-$  wherein  $m$  is an integer of from 1 to 3 and Aryl represents an aryl group of the benzene and naphthalene series, a bridge such as  $-\text{CONH}(\text{CH}_2)_n-$  wherein  $n$  has value given above,  $-\text{CONHCH}_2\text{CONH}(\text{CH}_2)_n-$  wherein  $n$  has the value given above, -succimido lower alkyl,  $-\text{NH}-\text{CO}(\text{CH}_2)_n-$  wherein  $n$  has the value given above,  $-\text{o-Aryl-CONH}(\text{CH}_2)_n-$  wherein Aryl and  $n$  have the values given above,



wherein Aryl and  $n$  have the values given above and X has the value given above.



wherein  $R_5$  represents hydrogen or lower alkyl;  $R_6$  represents an alkyl group which can be directly linked to the heterocyclic nucleus or through a  $-\text{CONH}-$  bridge; and  $R_7$  represents an alkyl group which can be substituted by aryl radicals of the benzene and naphthalene series, carbamyl radicals and carboxyalkoxy radicals, and one of said  $R_6$  and  $R_7$  always containing an alkyl group of at least 8 carbon atoms, V represents the non-metallic atoms necessary to complete a heterocyclic nucleus of the benzothiazole series, pyridine series, quinoline series and benzimidazole series and X has the value given above.



wherein  $R_1$  has the value given above;  $R_8$  can be hydrogen or alkyl,  $R_9$  can be alkyl or a heterocyclic nucleus of the pyridine, quinoline or benzothiazole series,  $p$  can be an integer of from 1 to 2; T can be a bridge such as



$-\text{CONH-Arylene-CONH}-$  wherein Arylene is a mono or bicyclic aromatic radical,  $-\text{o-Arylene-CO-}$  wherein Arylene has the values given above



wherein  $n$  has the value given above and  $-\text{SO}_2-$ ; and X has the value given above.



wherein Alk,  $R_1$  and X have the values given above.



wherein Alk,  $R_1$  and X have the values given above.

As previously pointed out, the photographic properties of a silver halide polyvinyl alcohol emulsion can be regulated by adjusting the electrical charge at or near the silver halide grains. Such a charge can be established by the adsorption of various surface-active agents at the silver halide surface. Although the aforesaid cationics make it possible to establish a positive charge of varying intensity around the light-sensitive silver halide grains, precise control of the photographic properties of the emulsion necessitates adjusting the negative charge as well. Thus, by the introduction into the cationic molecule of the various acidic groups of the type illustrated above, a structure is thereby produced having positive and negative seats or charges. By selecting the proper combination of negative and positive groupings, an amphoteric compound or amphotelyte can be produced capable of controlling the charge pattern and, therefore, the photographic properties of a polyvinyl alcohol silver halide emulsion with much greater precision than by means of the cationics alone.

In the following list are depicted various amphotelytes which are illustrative of the types used in accordance with this invention.

Aliphatic amino carboxylic acids and taurines having an alkyl radical of at least 8 carbon atoms.

Betaines of the formula:



wherein  $R_2$  and  $R_3$  have the values given above; K can be single carbon-carbon bond, a polymethylene bridge of from 1 to 4 carbon atoms, a linkage such as



wherein  $t$  is an integer of from 1 to 4



wherein  $t$  has the value given above,



wherein Alk has the value given above, CONH-Aryl— wherein Aryl has the value given above,  $\text{CH}_2-\text{o-Aryl}-$  wherein Aryl has the value given above,  $-\text{CO-Aryl}$  wherein Aryl has the value given above;  $R_{10}$  and  $R_{11}$  represent hydrogen, alkyl, one of which can be substituted by an amino group; and  $R_{10}$  and  $R_{11}$  together can complete a heterocyclic nucleus of the pyridine series;  $R_{12}$  can be an alkyl group attached directly to the quaternary nitrogen atom or through an intervening linkage (L) of the type described above for  $-\text{U}-$  under aliphatic quaternary ammonium compounds and one of  $R_{10}$ ,  $R_{11}$  and  $R_{12}$  always being an alkyl chain of at least 8 carbon atoms, T is an acid radical such as  $-\text{COOH}$ ,  $-\text{SO}_3\text{H}$ , or  $-\text{PO}_3\text{H}_2$  and X has the value given above.

Thetines of the formula:



wherein Alk,  $R_1$ , T and  $n$  have the values given above.



70 wherein  $R_1$ , Alk and  $n$  have the values given above.

All of the amphotelytic and cationic materials, of the type used herein, are provided with long chain or polymeric moieties to endow the molecules with surface-active properties which greatly influence their mode of adsorption on the silver halide grains. According to the photographic

literature, such surface-active agents are capable of displacing simple ions (e.g.,  $\text{Ag}^+$  or  $\text{Br}^-$ ) from the silver halide grain surface.

By properly selecting and applying the appropriate surface-active ampholytes or combinations of ampholytes and cationics, it is possible to control the type, number and distribution of charged sites on the silver halide grain surface.

The establishment of a predetermined charge arrangement on or about the silver halide grain not only facilitates grain growth and peptization, but regulates the subsequent adsorption of photographically active ions (sulfur sensitizers, gold sensitizers, stabilizers and developers, etc.) all of which have a profound influence on the photographic characteristics of the ripened, exposed and processed emulsions. Although such compounds possess similar cationic and anionic functional groups, the various auxiliary substituents, depending on their position in the molecule, markedly influence the degree of adsorption of the surface-active materials on the silver halide grain and thereby affect the physical and chemical ripening properties of the photographic emulsions prepared therefrom.

The application of the appropriate materials permits the preparation of polyvinyl alcohol emulsions possessing a selected range of grain sizes and therefore exhibiting a wide variety of speed and gradation characteristics.

In general, it has been observed that the surface-active cationics are difficult to apply because of their fogging tendencies, and can only be used for the preparation of low speed paper emulsions which are highly stabilized with synthetic antifoggants. The surface-active ampholytes, on the other hand, permit the greatest latitude in emulsion-making conditions, and can be applied over a wide concentration range without producing an undesirable fog level. In some instances, as will be described later, the ampholytes are advantageously used in combination with the cationics in order to bring out their maximum peptizing and sensitizing properties.

The following is a detailed list of the various activators which are useful in the preparation of the polyvinyl alcohol photographic silver halide emulsions described herein. In all the compounds, the chemical structure of each contains a polymeric moiety or an alkyl or alkylene chain of at least 8 carbon atoms.

Table I

## SURFACE-ACTIVE CATIONIC AGENTS

| Compound No.<br>(C=cationic) | Structure                                                                                                                                               |
|------------------------------|---------------------------------------------------------------------------------------------------------------------------------------------------------|
| C-1                          | $\text{RNH}_2$ ( $\text{R}=\text{C}_8\text{H}_{17}$ to $\text{C}_{18}\text{H}_{37}$ )                                                                   |
| C-2                          | $\text{C}_{18}\text{H}_{37}\text{NHCH}_3$                                                                                                               |
| C-3                          | $\text{C}_{14}\text{H}_{29}\text{N}(\text{CH}_3)_3$                                                                                                     |
| C-4                          | $\text{C}_{16}\text{H}_{33}\text{N}(\text{CH}_3)_3$                                                                                                     |
| C-5                          | $\text{C}_{18}\text{H}_{37}\text{N}(\text{CH}_3)_3$                                                                                                     |
| C-6                          | $\text{C}_8\text{H}_{17}-\text{C}_6\text{H}_4-\text{OCH}_2\text{CH}_2\text{OCH}_2\text{CH}_2-\text{N}(\text{CH}_3)_3$                                   |
| C-7                          | $\text{H}_2\text{NCH}_2\text{CH}_2-(\text{CH}_2)_{10}-\text{CH}_2\text{CH}_2\text{NH}_2$                                                                |
| C-8                          | $\text{CH}_2\text{CH}_2-\text{O}-\text{CH}_2\text{CH}_2-\text{N}-(\text{CH}_2)_{10}-\text{N}(\text{CH}_2\text{CH}_2-\text{O}-\text{CH}_2\text{CH}_2)_2$ |
| C-9                          | $\text{C}_4\text{H}_9-\text{N}-(\text{CH}_2)_{10}-\text{N}(\text{C}_4\text{H}_9)_2$                                                                     |
| C-10                         | $\text{C}_4\text{H}_9-\text{N}-(\text{CH}_2)_{10}-\text{N}(\text{C}_2\text{H}_5)_2$                                                                     |
| C-11                         | $\text{C}_{10}\text{H}_{21}-\text{CH}(\text{NH}_2)-\text{COOC}_2\text{H}_5 \cdot \text{HCl}$                                                            |
| C-12                         | $\text{C}_{10}\text{H}_{21}-\text{CH}(\text{NH}_2)-\text{CONH}_2 \cdot \text{HCl}$                                                                      |
| C-13                         | $\text{C}_{16}\text{H}_{33}\text{NH}-\text{COCH}_2-\text{N}(\text{CH}_3)_3$                                                                             |
| C-14                         | $\text{C}_{16}\text{H}_{33}\text{NH}-\text{COCH}_2-\text{N}(\text{C}_2\text{H}_5)_3$                                                                    |

Table I—Continued  
SURFACE-ACTIVE CATIONIC AGENTS

| Compound No.<br>(C=cationic) | Structure                                                                                                                                        |
|------------------------------|--------------------------------------------------------------------------------------------------------------------------------------------------|
| C-15.....                    | $\text{C}_7\text{H}_{15}\text{CONH}-(\text{CH}_2)_3\text{N} \begin{array}{c} \text{CH}_3 \\   \\ \text{CH}_3 \\   \\ \text{CH}_3 \end{array}$    |
| C-16.....                    | $\text{C}_9\text{H}_{19}\text{CONH}-(\text{CH}_2)_3\text{N} \begin{array}{c} \text{CH}_3 \\   \\ \text{CH}_3 \\   \\ \text{CH}_3 \end{array}$    |
| C-17.....                    | $\text{C}_{11}\text{H}_{23}\text{CONH}-(\text{CH}_2)_3\text{N} \begin{array}{c} \text{CH}_3 \\   \\ \text{CH}_3 \\   \\ \text{CH}_3 \end{array}$ |
| C-18.....                    | $\text{C}_{13}\text{H}_{27}\text{CONH}-(\text{CH}_2)_3\text{N} \begin{array}{c} \text{CH}_3 \\   \\ \text{CH}_3 \\   \\ \text{CH}_3 \end{array}$ |
| C-19.....                    | $\text{C}_{15}\text{H}_{31}\text{CONH}-(\text{CH}_2)_3\text{N} \begin{array}{c} \text{CH}_3 \\   \\ \text{CH}_3 \\   \\ \text{CH}_3 \end{array}$ |
| C-20.....                    | $\text{C}_{17}\text{H}_{35}\text{CONH}-(\text{CH}_2)_3\text{N} \begin{array}{c} \text{CH}_3 \\   \\ \text{CH}_3 \\   \\ \text{CH}_2 \end{array}$ |
| C-21.....                    | $\text{C}_{14}\text{H}_{29}\text{NH}-\text{CH}_2-\text{C}_6\text{H}_5$                                                                           |
| C-22.....                    | $(\text{CH}_2)_8 < \left( \text{CONH}(\text{CH}_2)_3-\text{N} \begin{array}{c} \text{CH}_3 \\   \\ \text{CH}_3 \end{array} \right)_2$            |
| C-23.....                    | $\text{C}_{17}\text{H}_{35}\text{CONH}-(\text{CH}_2)_2-\text{N} \begin{array}{c} \text{C}_2\text{H}_5 \\   \\ \text{C}_2\text{H}_5 \end{array}$  |
| C-24.....                    | $\text{C}_{15}\text{H}_{27}\text{CONH}-\text{C}_8\text{H}_8$                                                                                     |
| C-25.....                    | $\text{C}_6\text{H}_5-\text{NHCOOC}_{13}\text{H}_{27}$                                                                                           |
| C-26.....                    | $\left( \text{CH}_2-\text{CH}_2 \right)_n$<br>$\text{C}_6\text{H}_5$                                                                             |
| C-27.....                    | $\text{C}_8\text{H}_{17}\text{NH}-\text{C} \begin{array}{c} \text{NH} \\    \\ \text{NH}_2 \end{array} \cdot \text{HX}$                          |
| C-28.....                    | $\text{C}_{10}\text{H}_{21}\text{NH}-\text{C} \begin{array}{c} \text{NH} \\    \\ \text{NH}_2 \end{array} \cdot \text{HX}$                       |
| C-29.....                    | $\text{C}_{12}\text{H}_{25}\text{NH}-\text{C} \begin{array}{c} \text{NH} \\    \\ \text{NH}_2 \end{array} \cdot \text{HX}$                       |
| C-30.....                    | $\text{C}_{14}\text{H}_{29}\text{NH}-\text{C} \begin{array}{c} \text{NH} \\    \\ \text{NH}_2 \end{array} \cdot \text{HX}$                       |
| C-31.....                    | $\text{C}_{16}\text{H}_{33}\text{NH}-\text{C} \begin{array}{c} \text{NH} \\    \\ \text{NH}_2 \end{array} \cdot \text{HX}$                       |

Table I—Continued  
SURFACE-ACTIVE CATIONIC AGENTS

| Compound No.<br>(C=cationic) | Structure                                                                                                                                                         |
|------------------------------|-------------------------------------------------------------------------------------------------------------------------------------------------------------------|
| C-32                         | $\text{C}_{18}\text{H}_{37}\text{NH}-\text{C}(=\text{NH})-\text{NH}_2 \cdot \text{HX}$                                                                            |
| C-33                         | $\text{C}_{14}\text{H}_{20}\text{O}-\text{C}_6\text{H}_4-\text{NH}-\text{C}(=\text{NH})-\text{NH}_2 \cdot \text{HX}$                                              |
| C-34                         | $\text{C}_{12}\text{H}_{25}\text{NH}-\text{C}(=\text{NH})-\text{NH}-\text{C}(=\text{NH})-\text{NH}_2-2\text{HX}$                                                  |
| C-35                         | $\text{C}_{16}\text{H}_{33}\text{NH}-\text{C}(=\text{NH})-\text{NH}-\text{C}(=\text{NH})-\text{NH}_2-2\text{HX}$                                                  |
| C-36                         | $\text{C}_{16}\text{H}_{21}\text{O}-\text{C}_6\text{H}_4-\text{NH}-\text{C}(=\text{NH})-\text{NH}-\text{C}(=\text{NH})-\text{NH}_2-2\text{HX}$                    |
| C-37                         | $\left[ \text{C}_6\text{H}_4-\text{NH}-\text{C}(=\text{NH})-\text{NH}-\text{C}(=\text{NH})-\text{NH}_2 \right]_n$                                                 |
| C-38                         | $\text{C}_{16}\text{H}_{33}-\text{N}(\text{CH}_3)_2-\text{O}$                                                                                                     |
| C-39                         | $\text{C}_{16}\text{H}_{33}-\text{N}^+(\text{CH}_3)_2\text{X}^-$                                                                                                  |
| C-40                         | $\text{C}_{16}\text{H}_{33}-\text{N}^+(\text{CH}_2\text{C}_6\text{H}_4\text{X})_2$                                                                                |
| C-41                         | $\text{C}_{16}\text{H}_{33}-\text{N}^+(\text{CH}_2\text{C}_4\text{H}_9)_2\text{X}^-$                                                                              |
| C-42                         | $\text{C}_{16}\text{H}_{33}-\text{N}^+(\text{CH}_2\text{CONH}_2)_2\text{X}^-$                                                                                     |
| C-43                         | $\text{C}_{16}\text{H}_{33}-\text{N}^+(\text{CH}_2\text{COOC}_2\text{H}_5)_2\text{X}^-$                                                                           |
| C-44                         | $\text{C}_8\text{H}_{17}-\text{C}_6\text{H}_4-\text{OCH}_2\text{CH}_2\text{OCH}_2\text{CH}_2-\text{N}^+(\text{CH}_3)_2-\text{C}_6\text{H}_4-\text{CH}_2\text{Cl}$ |
| C-45                         | $\text{C}_7\text{H}_{15}\text{CONH}-\text{CH}_2-\text{N}^+(\text{CH}_3)_2\text{X}^-$                                                                              |
| C-46                         | $\text{C}_9\text{H}_{19}\text{CONH}-\text{CH}_2-\text{N}^+(\text{CH}_3)_2\text{X}^-$                                                                              |
| C-47                         | $\text{C}_{11}\text{H}_{23}\text{CONH}-\text{CH}_2-\text{N}^+(\text{CH}_3)_2\text{X}^-$                                                                           |
| C-48                         | $\text{C}_{15}\text{H}_{31}\text{CONH}-\text{CH}_2-\text{N}^+(\text{CH}_3)_2\text{X}^-$                                                                           |
| C-49                         | $\text{C}_{17}\text{H}_{35}\text{CONH}-\text{CH}_2-\text{N}^+(\text{CH}_3)_2\text{X}^-$                                                                           |

Table I—Continued  
SURFACE-ACTIVE CATIONIC AGENTS

| Compound No. (C = cationic) | Structure                                                                                                                                                                                                   |
|-----------------------------|-------------------------------------------------------------------------------------------------------------------------------------------------------------------------------------------------------------|
| C-50                        | $\text{C}_{15}\text{H}_{31}\text{CONH}-(\text{CH}_2)_3-\overset{\text{CH}_3}{\underset{\text{CH}_3}{\text{N}^+}}-\text{CH}_2\text{CONH}_2 \text{X}^-$                                                       |
| C-51                        | $\text{C}_{17}\text{H}_{35}\text{CONHCH}_2\text{CONH}-(\text{CH}_2)_3-\overset{\text{CH}_3}{\underset{\text{CH}_3}{\text{N}^+}}-\text{CH}_3 \text{X}^-$                                                     |
| C-52                        | $\text{C}_{15}\text{H}_{31}\text{CONH}-(\text{CH}_2)_3-\overset{\text{CH}_3}{\underset{\text{CH}_3}{\text{N}^+}}-\text{CH}_2\text{COOC}_2\text{H}_5 \text{X}^-$                                             |
| C-53                        | $\text{C}_{15}\text{H}_{31}\text{CONH}-(\text{CH}_2)_3-\overset{\text{CH}_3}{\underset{\text{CH}_3}{\text{N}^+}}-\text{CH}_2\text{CH}_2\text{CH}_2\text{COOC}_2\text{H}_5 \text{X}^-$                       |
| C-54                        | $\text{C}_{10}\text{H}_{19}-\text{CH}-\overset{\text{O}}{\text{C}}-\text{N}-(\text{CH}_2)_3-\overset{\text{CH}_3}{\underset{\text{CH}_3}{\text{N}^+}}-\text{CH}_2\text{CONH}_2 \text{X}^-$                  |
| C-55                        | $\text{C}_{10}\text{H}_{19}-\text{CH}-\overset{\text{O}}{\text{C}}-\text{N}-(\text{CH}_2)_3-\overset{\text{CH}_3}{\underset{\text{CH}_3}{\text{N}^+}}-\text{C}_2\text{H}_5 \text{X}^-$                      |
| C-56                        | $\text{CH}_2-\overset{\text{O}}{\text{C}}-\text{N}-(\text{CH}_2)_3-\overset{\text{CH}_3}{\underset{\text{CH}_3}{\text{N}^+}}-\text{CH}_2\text{CONH}\text{C}_{18}\text{H}_{37} \text{X}^-$                   |
| C-57                        | $\text{CH}_2-\overset{\text{O}}{\text{C}}-\text{N}-(\text{CH}_2)_3-\overset{\text{CH}_3}{\underset{\text{CH}_3}{\text{N}^+}}-\text{C}_{18}\text{H}_{33} \text{X}^-$                                         |
| C-58                        | $\text{CH}_3\text{CONH}-(\text{CH}_2)_3-\overset{\text{CH}_3}{\underset{\text{CH}_3}{\text{N}^+}}-\text{C}_{18}\text{H}_{33} \text{X}^-$                                                                    |
| C-59                        | $\text{C}_{18}\text{H}_{35}-\text{CH}-\overset{\text{O}}{\text{C}}-\text{N}-(\text{CH}_2)_3-\overset{\text{CH}_3}{\underset{\text{CH}_3}{\text{N}^+}}-\text{CH}_2\text{CO}-\text{C}_6\text{H}_5 \text{X}^-$ |
| C-60                        | $\text{C}_{16}\text{H}_{33}\text{NHCOCH}_2-\overset{\text{CH}_3}{\underset{\text{CH}_3}{\text{N}^+}}-\text{CH}_3 \text{X}^-$                                                                                |
| C-61                        | $\text{C}_{16}\text{H}_{33}\text{NHCOCH}_2-\overset{\text{C}_2\text{H}_5}{\underset{\text{C}_2\text{H}_5}{\text{N}^+}}-\text{CH}_2-\text{C}_6\text{H}_5 \text{X}^-$                                         |
| C-62                        | $\text{C}_{16}\text{H}_{33}-\text{NHCOCH}_2-\overset{\text{CH}_3}{\underset{\text{CH}_3}{\text{N}^+}}-\text{CH}_2\text{CO}-\text{C}_6\text{H}_5 \text{X}^-$                                                 |
| C-63                        | $\text{C}_{16}\text{H}_{33}\text{NHCOCH}_2-\overset{\text{C}_2\text{H}_5}{\underset{\text{C}_2\text{H}_5}{\text{N}^+}}-\text{CH}_2\text{COOC}_2\text{H}_5 \text{X}^-$                                       |
| C-64                        | $\text{C}_{16}\text{H}_{33}\text{NHCOCH}_2-\overset{\text{C}_2\text{H}_5}{\underset{\text{C}_2\text{H}_5}{\text{N}^+}}-\text{CH}_2\text{CH}_2\text{CH}_2\text{COOC}_2\text{H}_5 \text{X}^-$                 |

Table I—Continued  
SURFACE-ACTIVE CATIONIC AGENTS

| Compound No. (C = cationic) | Structure                                                                           |
|-----------------------------|-------------------------------------------------------------------------------------|
| C-65                        |    |
| C-66                        |    |
| C-67                        |    |
| C-68                        |    |
| C-69                        |    |
| C-70                        |    |
| C-71                        |   |
| C-72                        |  |
| C-73                        |  |
| C-74                        |  |
| C-75                        |  |
| C-76                        |  |

Table I—Continued  
SURFACE-ACTIVE CATIONIC AGENTS

| Compound No. (C = cationic) | Structure |
|-----------------------------|-----------|
| C-77                        |           |
| C-78                        |           |
| C-79                        |           |
| C-80                        |           |
| C-81                        |           |
| C-82                        |           |
| C-83                        |           |
| C-84                        |           |
| C-85                        |           |
| C-86                        |           |
| C-87                        |           |
| C-88                        |           |
| C-89                        |           |
| C-90                        |           |

Table I—Continued  
SURFACE-ACTIVE CATONIC AGENTS

| Compound No. (C = cationic) | Structure |
|-----------------------------|-----------|
| C-91                        |           |
| C-92                        |           |
| C-93                        |           |
| C-94                        |           |
| C-95                        |           |

Table II  
SURFACE-ACTIVE AMPHOLYTIC AGENTS

| Compound No. (A = amphotolyte) | Structure                                                                                              |
|--------------------------------|--------------------------------------------------------------------------------------------------------|
| A-1                            | C <sub>12</sub> H <sub>25</sub> NHCH <sub>2</sub> COOH                                                 |
| A-2                            | C <sub>16</sub> H <sub>33</sub> NHCH <sub>2</sub> COOH                                                 |
| A-3                            | C <sub>18</sub> H <sub>37</sub> NHCH <sub>2</sub> COOH                                                 |
| A-4                            | C <sub>12</sub> H <sub>25</sub> NHCH <sub>2</sub> CH <sub>2</sub> COOH                                 |
| A-5                            | C <sub>16</sub> H <sub>33</sub> NHCH <sub>2</sub> CH <sub>2</sub> COOH                                 |
| A-6                            | C <sub>16</sub> H <sub>33</sub> NH-(CH <sub>2</sub> ) <sub>3</sub> COOH                                |
| A-7                            | C <sub>16</sub> H <sub>29</sub> NH-(CH <sub>2</sub> ) <sub>5</sub> COOH                                |
| A-8                            | C <sub>12</sub> H <sub>25</sub> NH-CH <sub>2</sub> CH <sub>2</sub> SO <sub>3</sub> H                   |
| A-9                            | C <sub>18</sub> H <sub>37</sub> -N(CH <sub>3</sub> ) <sub>2</sub> CH <sub>2</sub> COOH                 |
| A-10                           | C <sub>10</sub> H <sub>21</sub> -CH(NH <sub>2</sub> )-COOH                                             |
| A-11                           |                                                                                                        |
| A-12                           |                                                                                                        |
| A-13                           | C <sub>16</sub> H <sub>33</sub> -N(CH <sub>2</sub> COOH) <sub>2</sub>                                  |
| A-14                           | C <sub>10</sub> H <sub>21</sub> -CH(NH-CH <sub>2</sub> COOH)-COOH                                      |
| A-15                           | C <sub>12</sub> H <sub>25</sub> N-CH <sub>2</sub> CH <sub>2</sub> N(CH <sub>2</sub> COOH) <sub>2</sub> |
| A-16                           | C <sub>10</sub> H <sub>21</sub> CH(NH-CH <sub>2</sub> CH <sub>2</sub> OH)-COOH                         |
| A-17                           | C <sub>10</sub> H <sub>21</sub> CH(NH <sub>2</sub> )-CONHCH <sub>2</sub> COOH                          |
| A-18                           | H <sub>2</sub> N-(CH <sub>2</sub> ) <sub>4</sub> -CH(NH <sub>16</sub> H <sub>33</sub> )-COOH           |

Table II—Continued

## SURFACE-ACTIVE AMPHOLYTIC AGENTS

| Compound No. (A = amphotolyte) | Structure                                                                                                                   |
|--------------------------------|-----------------------------------------------------------------------------------------------------------------------------|
| A-19                           | $\text{C}_{10}\text{H}_{21}\text{CH}(\text{NH}_2)\text{CONHCH}(\text{CH}_2\text{COOH})\text{COOH}$                          |
| A-20                           | $\text{CH}_3(\text{CH}_2)_4\text{CH}(\text{NH}_2)(\text{CH}_2)_{11}\text{COOH}$                                             |
| A-21                           | $\text{C}_{18}\text{H}_{35}\text{CH}(\text{COOH})\text{CH}_2\text{CONH}(\text{CH}_2)_3\text{N}(\text{CH}_3)_2$              |
| A-22                           | $\text{C}_{14}\text{H}_{24}\text{N}^+ \text{CH}_2\text{COO}^-$                                                              |
| A-23                           | $\text{C}_{16}\text{H}_{33}\text{N}^+ \text{CH}_2\text{COO}^-$                                                              |
| A-24                           | $\text{C}_{18}\text{H}_{37}\text{N}^+ \text{CH}_2\text{COO}^-$                                                              |
| A-25                           | $\text{C}_8\text{H}_{17} \text{OC}_2\text{H}_4\text{OC}_2\text{H}_4\text{OC}_2\text{H}_4\text{N}^+ \text{CH}_2\text{COO}^-$ |
| A-26                           | $\text{CH}_2\text{CH}_2\text{N}^+ \text{CH}_2\text{COO}^-$                                                                  |
| A-27                           | $\text{O} \text{CH}_2\text{CH}_2\text{N}^+ \text{CH}_2\text{COO}^-$                                                         |
| A-28                           | $\text{C}_{16}\text{H}_{33}\text{CH}_2\text{N}^+ \text{CH}_2\text{COO}^-$                                                   |
| A-29                           | $\text{C}_{10}\text{H}_{21}\text{CH}_2\text{N}^+ \text{CH}_2\text{CH}_2\text{OH}$                                           |
| A-30                           | $\text{C}_{16}\text{H}_{33}\text{N}^+ \text{CH}_2\text{COO}^-$                                                              |
| A-31                           | $\text{C}_{16}\text{H}_{33}\text{N}^+ \text{CH}_2\text{COO}^-$                                                              |
| A-32                           | $\text{C}_{10}\text{H}_{21}\text{CH}_2\text{N}^+ \text{C}_6\text{H}_5$                                                      |
| A-33                           | $\text{C}_{14}\text{H}_{29}\text{CH}_2\text{N}^+ \text{C}_6\text{H}_5$                                                      |
| A-34                           | $\text{C}_{16}\text{H}_{33}\text{CH}_2\text{N}^+ \text{C}_6\text{H}_5$                                                      |

Table II—Continued  
SURFACE-ACTIVE AMPHOLYTIC AGENTS

| Compound No. (A = ampholyte) | Structure                                                                                                                                                                                                                                                                                      |
|------------------------------|------------------------------------------------------------------------------------------------------------------------------------------------------------------------------------------------------------------------------------------------------------------------------------------------|
| A-35                         | $  \begin{array}{c}  \text{CH}_3 \\    \\  \text{C}_{16}\text{H}_{33}-\text{N}^+-\text{CH}-\text{COO}^- \\    \\  \text{CH}_3  \end{array}  \text{Cyclohexyl group}  $                                                                                                                         |
| A-36                         | $  \begin{array}{c}  \text{CH}_3 \\    \\  \text{C}_{10}\text{H}_{33}-\text{N}^+-\text{CH}-\text{COO}^- \\    \\  \text{CH}_3 \quad \text{CH}_2-\text{COOH}  \end{array}  $                                                                                                                    |
| A-37                         | $  \begin{array}{c}  \text{H}_2\text{N}-\text{(CH}_2)_4-\text{CH}-\text{COO}^- \\    \\  \text{C}_{10}\text{H}_{33}-\text{N}^+-\text{CH}_3 \\    \\  \text{CH}_3  \end{array}  $                                                                                                               |
| A-38                         | $  \begin{array}{c}  \text{CH}_3 \\    \\  \text{C}_7\text{H}_{15}\text{CONH}-\text{(CH}_2)_3-\text{N}^+-\text{CH}_2\text{COO}^- \\    \\  \text{CH}_3  \end{array}  $                                                                                                                         |
| A-39                         | $  \begin{array}{c}  \text{CH}_3 \\    \\  \text{C}_9\text{H}_{19}\text{CONH}-\text{(CH}_2)_3-\text{N}^+-\text{CH}_2\text{COO}^- \\    \\  \text{CH}_3  \end{array}  $                                                                                                                         |
| A-40                         | $  \begin{array}{c}  \text{CH}_3 \\    \\  \text{C}_{11}\text{H}_{23}\text{CONH}-\text{(CH}_2)_3-\text{N}^+-\text{CH}_2\text{COO}^- \\    \\  \text{CH}_3  \end{array}  $                                                                                                                      |
| A-41                         | $  \begin{array}{c}  \text{CH}_3 \\    \\  \text{C}_{13}\text{H}_{27}\text{CONH}-\text{(CH}_2)_3-\text{N}^+-\text{CH}_2\text{COO}^- \\    \\  \text{CH}_3  \end{array}  $                                                                                                                      |
| A-42                         | $  \begin{array}{c}  \text{CH}_3 \\    \\  \text{C}_{15}\text{H}_{31}\text{CONH}-\text{(CH}_2)_3-\text{N}^+-\text{CH}_2\text{COO}^- \\    \\  \text{CH}_3  \end{array}  $                                                                                                                      |
| A-43                         | $  \begin{array}{c}  \text{CH}_3 \\    \\  \text{C}_{17}\text{H}_{35}\text{CONH}-\text{(CH}_2)_3-\text{N}^+-\text{CH}_2\text{COO}^- \\    \\  \text{CH}_3  \end{array}  $                                                                                                                      |
| A-44                         | $  \begin{array}{c}  \text{CH}_3 \\    \\  \text{CH}_3(\text{CH}_2)_7-\text{CH}=\text{CH}-\text{(CH}_2)_7-\text{CONH}-\text{(CH}_2)_3-\text{N}^+-\text{CH}_2\text{COO}^- \\    \\  \text{CH}_3  \end{array}  $                                                                                 |
| A-45                         | $  \begin{array}{c}  \text{CH}_3 \\    \\  \text{CH}_3-(\text{CH}_2)_7-\text{CH}-\text{CH}(\text{OH})-\text{(CH}_2)_7-\text{CONH}-\text{(CH}_2)_3-\text{N}^+-\text{CH}_2\text{COO}^- \\    \\  \text{CH}_3  \end{array}  $                                                                     |
| A-46                         | $  \begin{array}{c}  \text{C}_2\text{H}_5 \\    \\  \text{C}_{17}\text{H}_{35}\text{CONH}-\text{CH}_2-\text{CH}_2-\text{N}^+-\text{CH}_2\text{COO}^- \\    \\  \text{C}_2\text{H}_5  \end{array}  $                                                                                            |
| A-47                         | $  \begin{array}{c}  \text{C}_{10}\text{H}_{19}-\text{CH}-\text{C}(=\text{O})-\text{CH}_2-\text{N}^+-\text{CH}_2\text{COO}^- \\    \quad   \\  \text{CH}_2-\text{C}(=\text{O})-\text{CH}_2 \quad \text{CH}_3 \\    \quad   \\  \text{C}_2\text{H}_5 \quad \text{C}_2\text{H}_5  \end{array}  $ |
| A-48                         | $  \begin{array}{c}  \text{C}_{15}\text{H}_{35}-\text{CH}-\text{C}(=\text{O})-\text{CH}_2-\text{N}^+-\text{CH}_2\text{COO}^- \\    \quad   \\  \text{CH}_2-\text{C}(=\text{O})-\text{CH}_2 \quad \text{CH}_3 \\    \quad   \\  \text{C}_2\text{H}_5 \quad \text{C}_2\text{H}_5  \end{array}  $ |
| A-49                         | $  \begin{array}{c}  \text{C}_{17}\text{H}_{35}\text{CONHCH}_2\text{CONH}(\text{CH}_2)_3\text{N}^+-\text{CH}_2\text{COO}^- \\    \\  \text{CH}_3  \end{array}  $                                                                                                                               |

Table II—Continued

## SURFACE-ACTIVE AMPHOLYTIC AGENTS

| Compound No. (A = amphotolyte) | Structure                                                                                                                                                                                                       |
|--------------------------------|-----------------------------------------------------------------------------------------------------------------------------------------------------------------------------------------------------------------|
| A-50                           | $\text{C}_{17}\text{H}_{35}\text{CONH}-(\text{CH}_2)_3-\overset{\text{CH}_3}{\underset{\text{CH}_3}{\text{N}^+}}-\overset{\text{CH}_3}{\underset{\text{CH}_3}{\text{C}^+-\text{COO}^-}}$                        |
| A-51                           | $\text{C}_{15}\text{H}_{31}\text{CONH}-\overset{\text{CH}_3}{\underset{\text{CH}_3}{\text{N}^+}}-\text{CH}_2\text{COO}^-$                                                                                       |
| A-52                           | $\text{C}_{17}\text{H}_{35}\text{CONH}-\overset{\text{CH}_3}{\underset{\text{CH}_3}{\text{N}^+}}-\text{CH}_2\text{COO}^-$                                                                                       |
| A-53                           | $\text{C}_{12}\text{H}_{25}\text{NHCOCH}_2-\overset{\text{C}_2\text{H}_5}{\underset{\text{C}_2\text{H}_5}{\text{N}^+}}-\text{CH}_2\text{COO}^-$                                                                 |
| A-54                           | $\text{C}_{16}\text{H}_{33}\text{NHCOCH}_2-\overset{\text{C}_2\text{H}_5}{\underset{\text{C}_2\text{H}_5}{\text{N}^+}}-\text{CH}_2\text{COO}^-$                                                                 |
| A-55                           | $\text{C}_{18}\text{H}_{37}\text{NHCOCH}_2-\overset{\text{C}_2\text{H}_5}{\underset{\text{C}_2\text{H}_5}{\text{N}^+}}-\text{CH}_2\text{COO}^-$                                                                 |
| A-56                           | $\text{C}_{16}\text{H}_{35}-\text{NH}-\text{COCH}_2-\overset{\text{CH}_3}{\underset{\text{CH}_3}{\text{N}^+}}-\text{CH}_2\text{COO}^-$                                                                          |
| A-57                           | $\text{C}_{18}\text{H}_{35}-\overset{\text{CH}_3}{\underset{\text{COOH}}{\text{CH}-\text{CH}_2}}-\text{CONH}-(\text{CH}_2)_3-\overset{\text{CH}_3}{\underset{\text{CH}_3}{\text{N}^+}}-\text{CH}_2\text{COO}^-$ |
| A-58                           | $(\text{CH}_2)_8=[\text{NH}(\text{CH}_2)_3-\overset{\text{CH}_3}{\underset{\text{CH}_3}{\text{N}^+}}-\text{CH}_2\text{COO}^-]_2$                                                                                |
| A-59                           | $(\text{CH}_2)_{10}=[\text{NH}(\text{CH}_2)_3-\overset{\text{CH}_3}{\underset{\text{CH}_3}{\text{N}^+}}-\text{CH}_2\text{COO}^-]_2$                                                                             |
| A-60                           | $\text{C}_{13}\text{H}_{27}\text{CONH}-\text{C}_6\text{H}_4-\text{CH}_2-\overset{\text{CH}_3}{\underset{\text{CH}_3}{\text{N}^+}}-\text{CH}_2\text{COO}^-$                                                      |
| A-61                           | $\text{C}_{16}\text{H}_{33}\text{O}-\text{C}_6\text{H}_4-\text{CONH}-(\text{CH}_2)_3-\overset{\text{CH}_3}{\underset{\text{CH}_3}{\text{N}^+}}-\text{CH}_2\text{COO}^-$                                         |
| A-62                           | $\text{C}_{11}\text{H}_{23}\text{CONH}-\text{C}_6\text{H}_4-\text{CONH}(\text{CH}_2)_3-\overset{\text{CH}_3}{\underset{\text{CH}_3}{\text{N}^+}}-\text{CH}_2\text{COO}^-$                                       |
| A-63                           | $\text{C}_{16}\text{H}_{31}\text{CONH}-\text{C}_6\text{H}_4-\text{CONH}(\text{CH}_2)_3-\overset{\text{CH}_3}{\underset{\text{CH}_3}{\text{N}^+}}-\text{CH}_2\text{COO}^-$                                       |
| A-64                           | $\text{C}_{11}\text{H}_{23}\text{CONH}-\text{C}_6\text{H}_4-\text{CONH}-(\text{CH}_2)_3-\overset{\text{CH}_3}{\underset{\text{CH}_3}{\text{N}^+}}-\text{CH}_2\text{COO}^-$                                      |
| A-65                           | $\text{C}_{15}\text{H}_{31}\text{CONH}-\text{C}_6\text{H}_4-\text{CONH}-(\text{CH}_2)_3-\overset{\text{CH}_3}{\underset{\text{CH}_3}{\text{N}^+}}-\text{CH}_2\text{COO}^-$                                      |

Table II—Continued  
SURFACE-ACTIVE AMPHOLYTIC AGENTS

| Compound No. (A = ampholyte) | Structure |
|------------------------------|-----------|
| A-66                         |           |
| A-67                         |           |
| A-68                         |           |
| A-69                         |           |
| A-70                         |           |
| A-71                         |           |
| A-72                         |           |
| A-73                         |           |
| A-74                         |           |
| A-75                         |           |
| A-76                         |           |
| A-77                         |           |
| A-78                         |           |
| A-79                         |           |
| A-80                         |           |
| A-81                         |           |

Table II—Continued  
SURFACE-ACTIVE AMPHOLYTIC AGENTS

| Compound No. (A = ampholyte) | Structure                                                                                                                                                                                      |
|------------------------------|------------------------------------------------------------------------------------------------------------------------------------------------------------------------------------------------|
| A-82.....                    | $\text{C}_{18}\text{H}_{37}\text{NHCOC}_2\text{H}_2-\overset{\text{CH}_3}{\underset{\text{CH}_3}{\text{N}^+}}-(\text{CH}_2)_3\text{NH}-\text{COCH}_2\text{CH}_2\text{COO}^-$                   |
| A-83.....                    | $\text{C}_{18}\text{H}_{35}\text{CH}-\text{CH}_2-\text{CONH}-(\text{CH}_2)_3-\overset{\text{CH}_3}{\underset{\text{CH}_3}{\text{N}^+}}-\text{C}_2\text{H}_5$<br>$\text{COO}^-$                 |
| A-84.....                    | $\text{C}_{10}\text{H}_{19}-\text{CH}-\text{CH}_2-\text{CONH}-(\text{CH}_2)_3-\overset{\text{CH}_3}{\underset{\text{CH}_3}{\text{N}^+}}-\text{CH}_2\text{CONH}_2$<br>$\text{COO}^-$            |
| A-85.....                    | $\left( \text{S}-\text{CH}_2-\text{CH}-\text{COO}^- \text{CH}_3 \right. \text{NHCOCH}_2-\overset{\text{CH}_3}{\underset{\text{CH}_3}{\text{N}^+}}-\text{C}_{16}\text{H}_{33} \left. \right)_2$ |
| A-86.....                    | $\text{C}_{16}\text{H}_{33}-\overset{\text{CH}_3}{\underset{\text{CH}_3}{\text{N}^+}}-\text{CH}_2\text{CONH}-\text{C}_6\text{H}_4-\text{COO}^-$                                                |
| A-87.....                    | $\text{C}_{16}\text{H}_{33}-\overset{\text{CH}_3}{\underset{\text{CH}_3}{\text{N}^+}}-\text{CH}_2\text{CH}_2-\text{O}-\text{C}_6\text{H}_4-\text{COO}^-$                                       |
| A-88.....                    | $\text{C}_{16}\text{H}_{33}-\overset{\text{CH}_3}{\underset{\text{CH}_3}{\text{N}^+}}-\text{CH}_2\text{CONH}-\text{C}_6\text{H}_4-\text{COO}^-$                                                |
| A-89.....                    | $\text{C}_{13}\text{H}_{27}\text{CONH}-(\text{CH}_2)_3-\overset{\text{CH}_3}{\underset{\text{CH}_3}{\text{N}^+}}-\text{CH}_2\text{CONH}-\text{C}_6\text{H}_4-\text{COO}^-$                     |
| A-90.....                    | $\text{C}_{17}\text{H}_{35}\text{CONH}-(\text{CH}_2)_3-\overset{\text{CH}_3}{\underset{\text{CH}_3}{\text{N}^+}}-\text{CH}_2\text{CONH}-\text{C}_6\text{H}_4-\text{COO}^-$                     |
| A-91.....                    | $\text{C}_{17}\text{H}_{35}\text{CONH}-(\text{CH}_2)_3-\overset{\text{CH}_3}{\underset{\text{CH}_3}{\text{N}^+}}-\text{CH}-\text{CO}-\text{NH}-\text{C}_6\text{H}_4-\text{COO}^-$              |
| A-92.....                    | $\text{C}_{17}\text{H}_{35}\text{CONH}-(\text{CH}_2)_3-\overset{\text{CH}_3}{\underset{\text{CH}_3}{\text{N}^+}}-\text{CH}_2-\text{C}_6\text{H}_4-\text{COO}^-$                                |
| A-93.....                    | $\text{C}_{16}\text{H}_{33}-\overset{\text{CH}_3}{\underset{\text{CH}_3}{\text{N}^+}}-\text{CH}_2\text{CO}-\text{C}_6\text{H}_4-\text{COO}^-$                                                  |
| A-94.....                    | $\text{C}_{16}\text{H}_{33}\text{SO}_2-\text{NH}-(\text{CH}_2)_3-\overset{\text{CH}_3}{\underset{\text{CH}_3}{\text{N}^+}}-\text{CH}_2\text{COO}^-$                                            |
| A-95.....                    | $\text{C}_{14}\text{H}_{24}-\text{S}^+-\text{CH}_2\text{COO}^-$<br>$\text{C}_2\text{H}_5$                                                                                                      |
| A-96.....                    | $\text{H}_2\text{N}-\overset{\text{CH}_3}{\underset{\text{NH}}{\text{C}-\text{NH}}}-(\text{CH}_2)_3-\text{CH}-\text{COOH}$<br>$\text{NH} \qquad \qquad \qquad \text{NHCOOC}_{11}\text{H}_{23}$ |
| A-97.....                    | $\text{C}_{16}\text{H}_{33}-\overset{\text{CH}_3}{\underset{\text{CH}_3}{\text{N}^+}}-\text{CH}_2\text{CH}_2\text{SO}_3^-$                                                                     |
| A-98.....                    | $\text{C}_{16}\text{H}_{33}-\overset{\text{CH}_3}{\underset{\text{CH}_3}{\text{N}^+}}-\text{CH}_2\text{CH}_2-\text{S}-\text{SO}_3^-$                                                           |

Table II—Continued  
SURFACE-ACTIVE AMPHOLYTIC AGENTS

| Compound No. (A = ampholyte) | Structure                                                                                                                           |
|------------------------------|-------------------------------------------------------------------------------------------------------------------------------------|
| A-99.....                    | $\text{C}_{12}\text{H}_{25}-\text{N}-\text{CH}_2-\text{CH}_2-\text{SO}_3\text{H}$<br>                                               |
| A-100.....                   | $\text{C}_{11}\text{H}_{23}\text{CONH}-\text{C}_6\text{H}_4-\text{SO}_2\text{NH}-\text{CH}_2-\text{N}^+-\text{CH}_2\text{COO}-$<br> |
| A-101.....                   | $\text{C}_{11}\text{H}_{23}-\text{C}-\text{N}^+-\text{CH}_2-\text{CH}_2\text{CH}_2\text{OCH}_2\text{COONa}$<br>                     |
| A-102.....                   | $\text{C}_{17}\text{H}_{35}-\text{C}-\text{N}^+-\text{CH}_2-\text{CH}_2\text{CH}_2\text{OH}$<br>                                    |

Table III

| Compound No. (S = Stabilizer) | Structure |
|-------------------------------|-----------|
| S-1.....                      |           |
| S-2.....                      |           |
| S-3.....                      |           |
| S-4.....                      |           |
| S-5.....                      |           |
| S-6.....                      |           |

Table III—Continued

| Compound No. (S = Stabilizer) | Structure |
|-------------------------------|-----------|
| 30                            |           |
| 35 S-7.....                   |           |
| 40 S-8.....                   |           |
| 45 S-9.....                   |           |
| 50 S-10.....                  |           |
| 55 S-11.....                  |           |
| 60 S-12.....                  |           |
| 65 S-13.....                  |           |
| 70 S-14.....                  |           |
| 75                            |           |

Table III—Continued

| Compound No. (S = Stabilizer) | Structure |
|-------------------------------|-----------|
| S-15                          |           |
| S-16                          |           |
| S-17                          |           |
| S-18                          |           |
| S-19                          |           |
| S-20                          |           |
| S-21                          |           |
| S-22                          |           |
| S-23                          |           |
| S-24                          |           |
| S-25                          |           |
| S-26                          |           |
| S-27                          |           |
| S-28                          |           |
| S-29                          |           |
| S-30                          |           |
| S-31                          |           |

Table III—Continued

| Compound No. (S = Stabilizer) | Structure |
|-------------------------------|-----------|
| 5                             |           |
| S-32                          |           |
| 10                            |           |
| S-33                          |           |
| 15                            |           |
| 20                            |           |
| S-34                          |           |
| 25                            |           |
| 30                            |           |
| S-35                          |           |
| 35                            |           |
| S-36                          |           |
| 40                            |           |
| S-37                          |           |
| 45                            |           |
| S-38                          |           |
| 50                            |           |
| S-40                          |           |
| 55                            |           |
| S-41                          |           |
| 60                            |           |
| S-42                          |           |
| 65                            |           |
| S-43                          |           |
| 70                            |           |
| S-44                          |           |
| 75                            |           |

Table III—Continued

| Compound No. (S = Stabilizer) | Structure |
|-------------------------------|-----------|
| S-45-----                     |           |
| S-46-----                     |           |
| S-47-----                     |           |
| S-48-----                     |           |
| S-49-----                     |           |
| S-50-----                     |           |
| S-51-----                     |           |
| S-52-----                     |           |
| S-53-----                     |           |
| S-54-----                     |           |

**GENERAL PROCEDURE AND DIRECTIONS  
FOR PREPARING POLYVINYL ALCOHOL  
SILVER HALIDE EMULSIONS**

The following four basic types of emulsions were selected for evaluation of the cationics (C), amphotolytes (A) and stabilizers (S) listed in Tables I, II and III, respectively.

- (1) Contact printing paper emulsions
- (2) Projection enlarging paper emulsions
- (3) Ammonia type emulsions
- (4) Negative "boiled" type emulsions

Detailed directions for preparing each type of emulsion are presented elsewhere in the application.

The emulsion making procedures are similar to those used for the preparation of gelatin emulsions, and employ accepted principles of physical and chemical ripening familiar to those skilled in the art. Briefly, silver nitrate solution is added to alkali halides dissolved in aqueous polyvinyl alcohol, and the resulting silver halide dispersion is subjected to a chemical ripening whereby the silver halide grains acquire their optimum light-sensitivity. Stabilizers and antifoggants may be added prior to the silver halide precipitation or during or after the subsequent chemical ripening stage. The finished emulsion is coated on a suitable support and then exposed and processed in the conventional manner.

To ensure that optimum results will be obtained from utilization of the synthetic additives described herein, a detailed account of the various factors which influence the characteristics of polyvinyl alcohol emulsions is presented.

- 5 Wherever possible, and for purposes of illustration, comparisons are made with the techniques used in the gelatin emulsion system.

**(1) Source of Polyvinyl Alcohol**

- 10 The polyvinyl alcohol, used in the preparation of the photographic emulsions described herein, is a medium viscosity type produced by the acid hydrolysis of polyvinyl acetate. Such materials are available on the commercial chemical market and are manufactured under a variety of trade names. As examples of commercial polyvinyl alcohol suitable for practicing this invention, mention is made of "Elvanol 90-25" sold by the E. I. du Pont de Nemours & Company and "Gelyatol 2/75" available from the Shawnigan Resins Corporation, P.O. Box 1531, Springfield 2, Mass.

Although synthetic polymeric silver halide carriers are not subject to variations in photographic properties to the extent of a natural substance such as gelatin, slight differences in photographic activity of various batches of polyvinyl alcohol, as purchased, may occur. In such cases, it may be necessary to make minor adjustments in the concentrations of the amphotolytic and/or cationic agents.

**(2) Quantity of Polyvinyl Alcohols**

- 30 In the preparation of most gelatin-silver halide emulsions, it is common practice to carry out the physical or Ostwald ripening (grain growth) in a small proportion of the required gelatin and to add the major quantity of the gelatin at some later stage of the emulsion making operation. It is well-known in the photographic art that the gelatin plays an important role in the physical ripening process and by its proper selection and use, it is possible to control the size and distribution of the silver halide grains.

- 40 Polyvinyl alcohol, on the other hand, is not as good a protective colloid as gelatin and it is essential to use most or all of the required polyvinyl alcohol in the physical ripening stage.

It will be noted in the formulae, which will be described later, that approximately 150 to 200.0 g. of a 12.0 to 45 15.0% aqueous solution of polyvinyl alcohol is needed to suspend the silver halide grains which are derived from 10.0 g. of silver nitrate. If the quantity of polyvinyl alcohol is reduced below 50.0 g. per 10.0 g. of silver nitrate, sedimentation of the silver halide grains usually occurs.

- 50 As previously stated, the amphotolytic/cation combinations, as herein disclosed, increase the silver halide carrying capacity of polyvinyl alcohol. For example, without the synthetic additives, it is possible to disperse in 150.0 g. of 12% polyvinyl alcohol, the silver chloride derived from only 2.5 g. of silver nitrate. However, after incorporation of the proposed amphotolytic/cationics, the quantity can be increased to approximately 20.0 g. of silver nitrate per 150.0 g. of 12% polyvinyl alcohol.

**(3) Selection of Surface-Active Amphotolytes and Cationics**

- In general, the amphotolytes serve as the primary means of regulating the electrical charge arrangement on the silver halide grains which ultimately determines the physical and chemical ripening response of the polyvinyl alcohol emulsions. In some instances, it may be necessary to supplement the amphotolytes with one or more of the cationics in order to obtain certain photographic properties which cannot be affected with the amphotolytes alone. However, the cationics, by themselves, produce very foggy emulsions unless large quantities of stabilizers and antifoggants are used in conjunction therewith in which case the emulsions are very slow and useful only for printing paper applications.

I have discovered that surface-active betaines containing 75 quaternary ammonium and carboxylic acid groups possess

excellent peptizing and physical ripening properties and are recommended for preparing all types of emulsions. The alpha betaines, in which one carbon atom separates the quaternary nitrogen and carboxylic acid functional groups, are especially applicable for the extreme speed emulsions, whereas the other members of the series, beta, gamma, delta, etc. betaines, are more suitable for the slow negative emulsions.

The surface-active amino acids listed in Table II, since they are not as efficiently activating (grain growth, peptizing and sensitizing) agents as the betaines, are recommended for preparing positive type and paper emulsions.

The surface-active betaines and cationics possessing one or more amide linkages as a part of their molecular structure can be usually applied over a relatively broad concentration range, a property which permits a wide latitude in emulsion making conditions. Since they have low peptizing properties, the alpha betaines of this class must, in order to realize their optimum activating characteristics, be used in combination with the cationics.

The optimum concentration of the amphotolytic/cationic combinations should be determined empirically for each type of emulsion. If the concentration of the additives is too low, sedimentation of the silver halide grains will occur; and if the concentration is too high, the fog level of the emulsion will be excessive. Generally, the low speed, fine grain emulsions require a higher concentration of the amphotolytic/cationics than do the high speed, coarse grained emulsions. Also, a wider cationic concentration range is permissible in the former than in the latter. For example:

Paper emulsion formulation #1 (refer to examples):



High speed formulation #4a (refer to examples):

Ampholyte: Structure above (0.01 M), 10.0 cc.  
Catonic: Structure above (0.01 M), 0.3 cc. to 0.6 cc.

Again, it should be emphasized that the low speed emulsions are more highly stabilized with the synthetic fog inhibitors than the high speed emulsions, and can consequently tolerate a higher concentration of the cat-ionics.

Some of the amphotropic materials are excellent peptizing and physical and chemical ripening agents, by themselves, e.g.,



and must be utilized in a specified concentration range to achieve the desired photographic emulsion characteristics.

On the other hand, as stated above, the amide containing alpha betaines, e.g.,



peptize rather poorly, per se, even at a very high concentration level (up to 50.0 cc. of 0.01 M solution/10.0 g. of silver nitrate), and they must be combined with the 75

surface-active cationics listed in Table I to ensure that the silver halide grains will be dispersed satisfactorily. In the latter case, the amphotolyte concentration range is not too critical, but the cationics must be used in a very narrow specified range. It should be noted that, when they are used in the high speed formulations, neither class of compounds is effective, alone.

In some instances, it is desirable to intentionally use a good peptizing amphotelyte such as



in a concentration range below which it alone will adequately peptize the grains, and to arrive at the desired physical and chemical emulsion characteristics by the supplemental addition of an appropriate amount of the surface-active cationics.

In the high speed "boiled" type emulsions, maximum grain growth is usually obtained when the concentration of the amphotytes and/or cationics is just sufficient for proper peptization of the grains. Beyond this critical amount, the grains become progressively finer and the fog level increases proportionately. Again, it should be mentioned that the fog can be controlled by the addition of the antifoggants and stabilizers which are listed in Table III.

In the lower limits of the amphotolytic/cationic concentration range, the grains possess a very broad distribution which is characterized by an emulsion possessing a high toe speed and flat gradation. The upper concentration limit produces emulsions of a smaller average grain size, but of somewhat narrower distribution; consequently, the characteristic curve exhibits a lower speed and steeper gradation. It is to be noted that a similar relationship between the gelatin concentration and the physical (Ostwald) ripening properties exists in the "boiled" type gelatin emulsion system. It is well-known, to those skilled in the art, that the largest grain sizes are produced when the gelatin concentration is reduced to a value which is near the minimum amount required for peptization of the grains.

Most of the surface-active amphotytic and cationic materials are useful for the purposes disclosed in this invention when the unbroken hydrophobic chain length varies from approximately 8 to 18 carbon atoms. Below 45  $C_8$ , adequate peptization of the grains cannot usually be obtained. In general, the compounds possessing the longer chain lengths ( $C_{14}$  to  $C_{18}$ ) are more effective 50 than those provided with the shorter chain radicals ( $C_{10}$  to  $C_{12}$ ), and they may be utilized in smaller amounts. The shorter chain compounds, on the other hand, permit a broader and less critical control of the emulsion making operations.

#### (4) *Blending of Components*

It is standard practice, in working with the gelatin emulsion system, to select and blend suitable gelatins for specific types of emulsions. This technique can be applied to the polyvinyl alcohol emulsion system when the desired emulsion characteristics cannot be obtained by the incorporation of single additives. The blend may be composed of one or more amphotolytes, one or more cationics, or a combination of both. The emulsions, except where indicated below, usually acquire characteristics which lay somewhere between the properties produced by the individual additives acting alone. For example:





In the above pairs, each of the individual compounds are peptizing agents in their own right. However, in the example,



neither are very active by themselves, but together produce an excellent peptizing grain growth promoting combination.

#### (5) Alkali Halide Concentration

All of the unwashed silver chloride emulsions are prepared with a slight excess of chloride ions, e.g., 4.0 g. of sodium chloride per 10.0 g. of silver nitrate.

The unwashed projection printing paper emulsions are prepared with slightly less than the stoichiometric quantity of potassium bromide (6.5 g. of potassium bromide per 10.0 g. of silver nitrate) and a slight excess of sodium chloride (0.45 g. of sodium chloride per 10.0 g. of silver nitrate).

The high speed washed emulsions may contain a considerable excess of potassium bromide (7.5 g. to 10.0 g. of potassium bromide) to facilitate the growth of large grains. This grain growth promoting method is also used in the gelatin emulsion system.

The amount of iodide may be varied from 0.05 g. of potassium iodide per 10.0 g. of silver nitrate in the paper emulsions to as high as 1.5 g. of potassium iodide per 10.0 g. of silver nitrate in the super speed emulsions. Generally, as in the gelatin emulsion system, the high iodide emulsions are faster in speed, flatter in gradation and possess a lower fog density than the corresponding low iodide emulsions. The amount of surface-active cationic material must be increased in proportion to the iodide content.

#### (6) Percolation Variations

In the gelatin emulsion system, it is standard practice to obtain the desired grain size and distribution by varying the rate of silver nitrate addition and/or dividing and adding the silver nitrate in several portions. This technique is likewise applicable to the polyvinyl alcohol emulsion system, although the response may be as great as with the gelatin emulsions. It should be emphasized, however, that it is important to select the appropriate components for the specific type of emulsions desired, and to use percolation variations chiefly for producing the minor changes in emulsion characteristics.

#### (7) Ripening Temperatures

All the emulsions disclosed in this application may be prepared in the temperature range from 30° C. to 90° C., the lower temperatures producing the finer grain sizes, and the higher temperatures, the coarser grains. The contact and projection printing paper emulsions may be physically ripening in the 30 to 50° C. range, whereas as the negative speed emulsions are best prepared at temperatures of 60° C. or higher.

The chemical ripening phase of the emulsion making operation is carried out at 50° C. for a period of 30 minutes to 1.0 hour.

#### (8) Rate of Agitation

The equipment in which the polyvinyl alcohol emulsions are prepared comprises stainless steel vessels which

have been provided with a mechanical stirring device rotating at 200.0 r.p.m.

Trial runs have indicated that a variation in stirring rate will affect the emulsion characteristics. A slow rate of agitation favors the formation of larger grains, and produces emulsions which are faster in speed, flatter in gradation, and higher in fog density than when a faster rate is used.

The rate of agitation was found to be of considerable importance during the preparation of silver chloride emulsions from which the amphotolytic/cationic activating agents were omitted. It was observed that, if the rate of stirring was reduced to 25.0 r.p.m. during the silver nitrate addition, and then increased to its normal rate of 200.0 r.p.m. after a prescribed pause period, it was possible to obtain an increase in emulsion speed. The emulsion sensitivity and fog level increased in proportion to the duration of the pause. The observed behavior is probably due to the fact that a slight excess of Ag<sup>+</sup> ions is maintained momentarily in the emulsion during the slow rate of agitation. A positive charge is thus produced on the grain surface which causes a grain growth in the silver halide.

#### (9) Washing of Polyvinyl Alcohol Emulsions

In the gelatin emulsion system, the removal of unwanted salts can be accomplished by two general methods:

- (a) The emulsion is cooled, gelled, shredded, and washed in running water to a specified conductivity.
- (b) The liquid emulsion is precipitated with inorganic salts, and the emulsion particles are washed by decantation.

Polyvinyl alcohol does not form a thermoreversible gel like gelatin, and consequently it is essential to use precipitation method (b) as one of the means of removing the soluble salts.

It is known in the art that polyvinyl alcohol emulsions can be temporarily insolubilized by precipitation with certain inorganic salts such as sodium or ammonium sulfate and can then be subjected to a wash treatment. The size and hardness of the precipitated particle depends on the type, concentration, and temperature of the precipitating solution, and on the rate at which it is added to the polyvinyl alcohol emulsion. Ammonium sulfate produces a tougher precipitate than does sodium sulfate; whereas, mixtures of the two reagents produce particles of intermediate hardness. If the emulsion is agitated slowly during the insolubilization treatment, it is transformed into a gelatinous mass which must be torn apart and shredded by hand before it can be washed.

Small particles can usually be obtained by:

- (a) Diluting the emulsion with water before precipitation,
- (b) Decreasing the rate of addition of the precipitating solution,
- (c) Increasing the rate of agitation, and by
- (d) Decreasing the temperature of the emulsion before precipitation.

Polyvinyl alcohol emulsions, which are precipitated in hard particles, withstand a vigorous wash treatment over a period of several hours, but, as a rule, become over-washed on the surface without being washed adequately in the center of the particle. On the other hand, emulsions which are precipitated in the form of soft particles become partially solubilized before the water soluble salts are removed completely.

The precipitation of the polyvinyl alcohol emulsions is carried out, in practice, by adding one of the following solutions to the high speed formulations described subsequently.

- (a) Sodium sulfate (20.0%), 350.0 cc.  
or
- (b) Ammonium sulfate (40.0%), 200.0 cc.  
or
- (c) Mixtures of (a) and (b).

The shredded emulsion is placed in a container, covered with a double thickness of cheesecloth, and washed with a slow but constant stream of filtered 20° C. tap water which is run in from a tube extending to the bottom of the container. The particles are thoroughly washed in about 2.0 to 3.0 hours. In most cases, the washed and drained emulsion weighs between 230.0 and 240.0 g. The emulsion is brought up to weight (250.0 g.) with water or 5.0% of polyvinyl alcohol, depending on the viscosity desired. Occasionally, when the emulsion is not precipitated hard enough and/or the wash period is too extended, the total weight, due to absorbed water, will vary between 260.0 and 320.0 g.

The emulsion is brought back into the liquid state by subjecting it to a "melting down" period. The time and temperature for an emulsion, which has been precipitated to such a degree of hardness and particle size that it can be washed for 2 to 3 hours, is 30 minutes at 70° C. A shorter time and lower temperature will result in incompletely dispersed emulsions. In those cases where softer precipitated particles are obtained, the temperature may be lowered to approximately 65° C.

Because of the difficulty in obtaining polyvinyl alcohol emulsion particles of uniform size and hardness, the precipitation method of washing polyvinyl alcohol emulsions has been displaced by the dialysis washing procedure. This technique can be applied to the polyvinyl alcohol emulsion system because, unlike gelatin emulsions, the polyvinyl alcohol silver halide dispersions are liquid at room temperature or lower.

The dialysis purification is accomplished very simply by pouring the emulsion into parchment paper or cellophane containers (each holding approximately 300.0 g. of emulsion), and immersing them in a tank through which a slow but constant stream of fresh 15 to 20° C. water is flowing. The emulsion, which is stirred constantly during the dialysis period, is completely washed in about 15.0 hours. If desired, the extent of soluble salt removal may be followed by conductivity measurements.

As soon as the dialysis is complete, the polyvinyl alcohol emulsion is ready for the chemical ripening phase of the emulsion making operation. As will be obvious to those skilled in the art, appropriate adjustments may have to be made in the pAg of the emulsion, since more than the requisite amount of soluble bromide ions may have been removed if the washing period is not controlled.

#### 10. Chemical Ripening of Polyvinyl Alcohol Emulsions

It is generally accepted that certain impurities, which are present in gelatin, are responsible for the chemical ripening of the silver halide emulsions. These materials are called labile sulfur compounds, because, under specified conditions of pH and temperature, they will react with silver halide to produce silver sulfide. It has been proposed that the presence of silver sulfide specks on the surface of the silver halide crystals is, in some way, responsible for the extreme light sensitivity of the grains.

Among the substances, which have been disclosed in the literature as chemical ripening agents, are sodium thiosulfate, sodium tetrathionate, thiourea and thioamide derivatives. In the polyvinyl alcohol emulsion system, it has been observed that sodium thiosulfate is as effective as most of the labile sulfur compounds, and consequently it has been used in the majority of the emulsion making experiments described therein.

As stated previously, none of the so called "inert" polyvinyl alcohol emulsions respond appreciably to chemical ripening reagents, although the experiments may be conducted over a wide pH and temperature range. However, the polyvinyl alcohol emulsions, which are prepared with the ampholytic/cationic combinations according to the disclosures in this invention, can be ripened with sodium thiosulfate to increase sensitivity in the manner of the conventional gelatin emulsions. The observed speed increase is 10 to 100 times over that of the chemically un-

ripened emulsion, with the contrast and maximum density increasing proportionately.

The quantity of sodium thiosulfate required depends on the type of emulsion, on the quantities of incorporated ampholytic/cationic materials, and on quantity of antifoggant which is added to the emulsion for stabilization purposes. In general, the high speed emulsions, which have a low stabilizer content, respond well to very small quantities of sodium thiosulfate (0.5 cc. to 2.0 cc. of 0.001 M solution per 100.0 g. of emulsion); whereas, the low speed, more highly stabilized emulsions require a somewhat larger amount (1.0 cc. to 5.0 cc. of 0.001 M solution per 100.0 g. of emulsion).

The chemical ripening process is carried out at 50° C. over a period of 30 minutes to 1.0 hour.

The sodium thiosulfate, or any other chemical ripening agent, may be added at any stage of the emulsion making procedure, but best results have always been obtained when the chemical ripening is carried out after the emulsion is washed free of excess soluble salts.

The high speed emulsions give the best response to labile sulfur ripening, and the projection paper emulsions the least. Ordinarily, the unwashed silver chloride emulsions are not subjected to chemical ripening.

#### 11. Gold Sensitization of Polyvinyl Alcohol Emulsions

It has been observed that the activated polyvinyl alcohol emulsions, which are disclosed herein, respond well to sensitization by gold salts and complexes in the same manner as the conventional gelatin emulsions. Gold sensitization is carried out during the chemical ripening stage, and results in a 1.0 to 1½ stop speed increase over that produced by chemical ripening, alone.

An ammonium aurous thiocyanate solution is prepared by adding 0.1 cc. of auric chloride solution (contains 40.0% of gold) to 100.0 cc. of ammonium thiocyanide (1.0%), and diluting the resulting solution to 1.0 liter with water. A quantity of 0.4 cc. to 1.2 cc. of the preceding gold solution is used per 100.0 g. of polyvinyl alcohol emulsion.

#### 12. Stabilization of Polyvinyl Alcohol Emulsions

All photographic emulsions, whether prepared from polyvinyl alcohol or gelatin, exhibit a tendency to acquire an undesirable fog density unless special precautions are taken to prevent its formation. The fog may be produced during the physical or chemical ripening stage of the emulsion making process or during the storage of the finished product.

It has been pointed out that the surface-active ampholytic and cationic materials must be incorporated in sufficient quantities to ensure an adequate peptization of the silver halide grains. Unfortunately, the fog level of the emulsion increases in proportion to the concentration of the activating compounds, and it is not always possible to obtain the desired size and distribution of the grains, as well as optimum chemical ripening by using a minimum quantity of the additives. From a practical standpoint, it is desirable to be able to use the activators over a broad concentration range. It is one of the functions of a satisfactory stabilizer to permit a wide latitude in emulsion making conditions.

Because the adsorbed surface-active ampholytes and cationics impart a positive charge on the silver halide grain surface, the stabilizer or antifoggant may function by partially displacing, neutralizing or "masking" some of the positive sites. It is also believed, according to the classical concepts of emulsion stabilization, that the stabilizer has the ability to regulate the  $\text{Ag}^+$  ion concentration of the emulsion by forming silver salts or complex ions of extremely low stability.

An examination of the structures of the stabilizers listed in Table III will reveal that all of them contain the weakly acidic  $-\text{SH}$ ,  $>\text{NH}$ , or  $-\text{OH}$  groups, or liberate these groups upon hydrolysis during ripening or storage. Com-

pounds S-1 to S-10 are the conventional stabilizers of the type commonly described in the photographic literature; whereas, compounds S-11 to S-39 are the conventional stabilizers which have been modified with long chain radicals. The long chain stabilizers have slightly different properties than the ordinary stabilizers because they are probably adsorbed more strongly on the grain surface than the latter. When added in excess amounts, the long chain materials appear to flatten the gradation of the emulsion before desensitizing the toe portion of the characteristic curve.

Some of the stabilizers such as compounds S-41 to S-49 in Table III contain both a long chain radical and a quaternary ammonium group in the same molecular structure. These substances were synthesized and evaluated in an attempt to reduce the inherent fogging characteristics of the surface-active cationic materials. It was observed, however, that the dual-functional compounds are desensitizing and they can be used only for blending purposes, or alone for the preparation of low speed emulsions.

There is also included in Table III some typical anionic surface-active materials such as compounds S-50 to S-55. These compounds are not antifoggants in the classical sense, and they probably function in the polyvinyl alcohol emulsion system by competing with the amphotolytic/cationic combinations for a place on the crystal surface. They are useful for making "minor" adjustments in the emulsion characteristics.

It is to be noted that the long chain guanidine and biguanide derivatives are unique in that they are basically desensitizing in nature, but when used in combination with the surface-active amphotolytes, they function as typical cationics. This behavior is probably due to the fact that the guanidines and biguanides form insoluble salts (U.S.P. 2,704,710) with the  $-\text{COOH}$  group in the amphotolyte and they shift the inner salt or "zwitterion" equilibrium so that there is a slight preponderance of the cationic, i.e., quaternary ammonium, functional group.

The long chain amphotolytes and cationics, which contain an amide functional group, also possess mild antifoggant and stabilizing properties in addition to their peptizing and grain promoting characteristics. The stabilizing behavior of the amide linkage can be attributed to a tautomerism in which a weakly acidic enol tautomer exhibiting antifogging properties is produced.



The ratio of enol to keto form is influenced by neighboring substituents in the molecule, and by the ability of the enol form to participate in inner salt formation. For example, the stabilizing effect is more pronounced in aromatic carboxamides and in carboxamides which are adjacent to quaternary nitrogen groups than in the straight aliphatic amides.



A sulfonamide linkage in the amphotolyte or cationic structure resembles the carboxamide linkage in its stabilizing and fog inhibiting properties.

The stabilizer selection and evaluation has been done on an empirical basis. In evaluating the emulsion trials, it has been observed that an insufficient quantity of the stabilizing or fog inhibiting substance will result in emulsions possessing both a high speed and high fog level. Conversely, an excess of stabilizer will produce a slow, but clean emulsion because of its inhibiting effect on the chemical ripening process.

The synthetic stabilizers and antifoggants in Table III may be added at any stage of the emulsion making operation. However, if they are incorporated prior to the silver nitrate addition, appropriate modifications have to be made to compensate for any changes which may occur in the degree of peptization and the growth of the grains.

As already stated, the low speed paper emulsions are activated with large quantities of the fog producing cationics and are, therefore, heavily stabilized to compensate for the rise in fog level. Approximately 2.0 to 5.0 cc. of a 0.01 M stabilizer solution is required per 100.0 g. of emulsion.

The washed high speed negative emulsions are low in cationic content and, therefore, require considerably less stabilizer than the paper emulsions. Generally, 0.2 to 1.0 cc. of a 0.01 M solution per 100.0 g. of emulsion is sufficient.

The negative type emulsions require great care in their preparation and extreme speed can only be attained by a very precise control of all the emulsion making variables, i.e., the type and quantity of amphotolyte/cationic, chemical ripening and stabilizing agents.

Among the simplest, yet most effective, ripening controls and fog inhibiting agents for high-speed emulsions are bromide or iodide ions. In the emulsion making process, it is essential to wash out all the unwanted soluble salts by precipitation or dialysis, and, as a result, the adsorbed bromide ion concentration may fall below a safe level. The soluble halide ion concentration may be readjusted by the addition of 1.0 to 2.0 cc. of 1.0% potassium bromide or 0.5 to 1.0 cc. of 1% potassium iodide per 100.0 g. of emulsion during the chemical ripening step.

The prevention of storage fog in the high speed polyvinyl alcohol emulsions is accomplished by the incorporation of a sodium benzenesulfinate solution containing traces of an organic disulfide as disclosed by F. W. H. Mueller in U.S. Patents 2,057,764; 2,394,198; 2,438,716; 2,440,110 and 2,440,206. Approximately 2.0 cc. of a 20.0% of sodium benzenesulfinate solution per 100.0 g. of emulsion is required.

### (13) Ammonia Type Emulsions

Ammonium hydroxide is an excellent physical ripening agent in the gelatin emulsion system and is useful for preparing the large grained, extreme speed, high contrast emulsions of the screen X-ray type at temperatures as low as 55° C. In the polyvinyl alcohol emulsion system, this is not the case, for, although ammonium hydroxide is an effective peptizing agent, it does not promote grain growth to any appreciable extent even at temperatures as high as 70° C.

An unmodified washed ammonia type polyvinyl alcohol emulsion has the speed of a projection enlarging paper, but after the incorporation of the amphotolytic/cationic combinations, labile sulfur compounds and gold complexes, it can be physically and chemically ripened to low speed negative emulsion. The long chain guanidine derivatives are among the most useful cationics for this purpose.

Because of the increased carrying capacity of polyvinyl alcohol for silver halide grains prepared by the ammonia process, it is possible to increase the silver to polyvinyl alcohol ratio considerably above that for the same emulsion prepared by the "boiled" process.

(14) *Optical Sensitization of Polyvinyl Alcohol Emulsions*

In general, the optical sensitization of polyvinyl alcohol silver halide photographic emulsions, prepared in accordance with this invention, involves techniques and procedures that are analogous to gelatin emulsions. Thus, sensitizing dyes known to be effective in a silver halide gelatin emulsion can ordinarily be used in the polyvinyl alcohol emulsion system.

Extensive investigations on the mechanism of optical sensitization in the polyvinyl alcohol emulsion system have indicated that there is a definite relationship between the electrical charge on the surface of the silver halide grains and the type and degree of optical sensitization. It is significant that second order sensitization is facilitated when the silver halide grains are prepared in the presence of or treated with the surface-active ampholytes and cationics as described herein.

(15) *Coating and Processing of Polyvinyl Alcohol Emulsions*

The polyvinyl alcohol silver halide emulsions described herein were dip coated using a double weight baryta raw paper stock or a suitably subbed cellulose ester film base for a support.

After exposure, the coatings were developed in the conventional negative developers such as Ansco Permadol, Normadol, Isodol, Formula #47 or #17, or paper developers such as Ansco Vividol or Formula #125.

Ansco Formula #125 has the following composition:

|                          | G.    |
|--------------------------|-------|
| Hot water                | 750.0 |
| Metol                    | 3.0   |
| Sodium sulfite           | 44.0  |
| Hydroquinone             | 12.0  |
| Sodium carbonate         | 65.0  |
| Potassium bromide        | 2.0   |
| Water to make 1.0 liter. |       |

For paper emulsions, the above formula is diluted with 2.0 liters of water and development is carried out at 20° C. for 1.0 to 2.0 minutes. For high speed polyvinyl alcohol emulsions, the formula is diluted with equal parts of water and development is carried out at 20° C. for 3.0 to 5.0 minutes.

All of the polyvinyl alcohol emulsions described herein can be developed and fixed and generally processed without the need of a hardening agent. However, if the processed paper coatings are dried at elevated temperatures, such as on a hot ferotyping drum, a hardener is required in order to prevent remelting of the polyvinyl alcohol. A hardening agent suitable for incorporation in polyvinyl alcohol emulsions is a melamine-formaldehyde resin of the type disclosed in U.S. Patents 2,367,511 and 2,691,604. Alternately, hardening of the coated emulsion can be accomplished by briefly rinsing the coatings in a 2.0 to 5.0% borax solution prior to placement on the ferotyping drum.

## EXAMPLES

In the examples listed below are presented detailed directions for the preparation of four basic types of photographic emulsions employing polyvinyl alcohol as the silver halide carrier. These examples are inserted for the purpose of illustration only and it is to be understood that the invention is not to be restricted thereto.

The ampholytes, cationics and stabilizers used in the examples were selected from Tables I, II and III. The following representative list of compounds can be used interchangeably in the concentration ranges cited in the formulations below.

Ampholytes: A-6, 24, 43, 49, 70, 71, 75, 78, 79, 83 and 94

Cationics: C-4, 19, 29, 39, 48, 51, 83 and 84

Stabilizers: S-1, 3, 4, 27, 30 and 37

The unwashed paper formulae were derived chiefly for convenience, and, if desired, they may be converted to the washed type by making appropriate changes in the formulations.

It is to be understood that the quantity of additives, which are recommended in the formulations, were found to be optimum for the emulsion making materials, equipment and conditions as described herein. It is obvious to those skilled in the art, that slight variations in the emulsion making procedures may alter the photographic properties of the emulsions.

Example #1.—*Unwashed Contact Printing Paper Emulsions*

## Part I:

|                                   |         |       |
|-----------------------------------|---------|-------|
| Gelvatol 2/75 (12.0%)             | -----g  | 150.0 |
| Sodium chloride (10.0%)           | -----cc | 40.0  |
| Ampholyte (0.01 M) see above list | -----cc | 10.0  |
| Cationic (0.01 M) see above list  | -----cc | 8.0   |

## Part II:

|                |         |      |
|----------------|---------|------|
| Silver nitrate | -----g  | 10.0 |
| Water          | -----cc | 70.0 |

Part II is added to Part I over a period of 1 to 30 minutes at a temperature of 50° C., and the resulting silver chloride dispersion is allowed to digest for 30 minutes at 50° C. To 100.0 g. of emulsion are added the following components:

|                                 |       |              |
|---------------------------------|-------|--------------|
| Optical sensitizing dye (0.05%) | ----- | 1.0-10.0 cc. |
| Stabilizer S-1 (0.5%)           | ----- | 0.6-1.2 cc.  |
| and                             |       |              |
| Stabilizer S-3 (0.01 M)         | ----- | 2.0-5.0 cc.  |
| or                              |       |              |
| Stabilizer S-4 (0.1%)           | ----- | 2.0-5.5 cc.  |
| 35 Saponin (8.0%)               | ----- | 1.6 cc.      |
| Water                           | ----- | As required  |

The coated emulsions, when processed as described above, possess photographic characteristics comparable to typical contact printing paper emulsions of the gelatin-silver halide system such as the Ansco Convira, Lustrex or Monodex products.

Example #2.—*Unwashed Projection Printing Paper Emulsions*

## Part I:

|                                   |         |          |
|-----------------------------------|---------|----------|
| Gelvatol 2/75 (12.0%)             | -----g  | 150.0    |
| Potassium bromide (50.0%)         | -----cc | 13.0     |
| Sodium chloride (10.0%)           | -----cc | 4.5      |
| Potassium iodide (10.0%)          | -----cc | 0.0-0.5  |
| Ampholyte (0.01 M) see above list | -----cc | 5.0-10.0 |
| Cationic (0.01 M) see above list  | -----cc | 2.0      |

## Part II:

|                |         |      |
|----------------|---------|------|
| Silver nitrate | -----g  | 10.0 |
| Water          | -----cc | 50.0 |

Part II is added to Part I over a period of 1 to 30 minutes at a temperature of 50° C., and the whole is allowed to digest at 50° C. for 30 minutes. The following components are added per 100.0 g. of emulsion and the emulsions are then ripened at 50° C. for 30 minutes:

|                              |       |             |
|------------------------------|-------|-------------|
| Sodium thiosulfate (0.001 M) | ----- | 1.0-5.0 cc. |
| Stabilizer S-3 (0.01 M)      | ----- | 2.0-5.0 cc. |
| or                           |       |             |
| Stabilizer S-4 (0.1%)        | ----- | 2.0-5.0 cc. |
| 65 Stabilizer S-37 (0.01 M)  | ----- | 2.0-5.0 cc. |
| Saponin (8.0%)               | ----- | 1.6 cc.     |
| Water                        | ----- | As required |

The coated emulsions, when processed as described above, possess photographic characteristics comparable to typical projection enlarging papers of the gelatin emulsion system such as Ansco Jet, Cykora or Indiatone paper products.

## Example #3.—Washed "Ammonia Type" Emulsions

## Part I:

|                                    |    |           |
|------------------------------------|----|-----------|
| Elvanol 90-25 (12.0%)              | g  | 150.0     |
| Potassium bromide (50.0%)          | cc | 15.0-20.0 |
| Potassium iodide (10.0%)           | cc | 4.0       |
| Ampholyte (0.01 M), see above list | cc | 5.0       |
| Cationic, C-29 (0.01 M)            | cc | 1.0-2.0   |

## Part II:

|                            |    |      |
|----------------------------|----|------|
| Silver nitrate             | g  | 10.0 |
| Ammonium hydroxide (28.0%) | cc | 10.0 |
| Water                      | cc | 40.0 |

Part II is added to Part I over a period of 1 to 30 minutes at a temperature of 50 to 70° C., and the whole is allowed to digest for 30 minutes at a temperature of 50 to 70° C. The emulsions are washed by dialysis for 15 hours at 2° C. according to the procedure described above. The following components are added per 100.0 g. of emulsion and the emulsions are then ripened at 50° C. for 30 minutes:

|                                             |              |
|---------------------------------------------|--------------|
| Sodium thiosulfate (0.001 M)                | 0.5-2.0 cc.  |
| Sodium benzenesulfinate (20.0%)             | 2.0 cc.      |
| Gold solution (prepared as described above) | 0.8 cc.      |
| Potassium iodide (1.0%)                     | 0.5-1.0 cc.  |
| or                                          |              |
| Potassium bromide (1.0%)                    | 1.0-2.0 cc.  |
| and/or                                      |              |
| Stabilizer S-3 (0.01 M)                     | 0.2-1.0 cc.  |
| and/or                                      |              |
| Stabilizer S-27 (0.01 M)                    | 0.2-1.0 cc.  |
| and/or                                      |              |
| Stabilizer S-30 (0.01 M)                    | 0.2-1.0 cc.  |
| and/or                                      |              |
| Stabilizer S-37 (.01 M)                     | 0.2-1.0 cc.  |
| Prior to coating, there is added:           |              |
| Optical sensitizing dye (0.05%)             | 1.0-10.0 cc. |
| Saponin (8.0%)                              | 1.6 cc.      |
| Water                                       | As required. |

The coated emulsions, when processed as described above, possess photographic characteristics comparable to typical slow negative emulsions of the gelatin emulsion system such as Ansco Commercial, Commercial Ortho, or Process films.

## Example #4.—Washed Negative High Speed "Boiled Type" Emulsions

## Part Ia (alternative):

|                                    |    |           |
|------------------------------------|----|-----------|
| Elvanol 90-25 (15.0%)              | g  | 200.0     |
| Potassium bromide (50.0%)          | cc | 15.0-20.0 |
| Potassium iodide (10.0%)           | cc | 2.0-8.0   |
| Ampholytes: A-43, 49, or 94        | cc | 5.0-20.0  |
| Cationics: (0.01 M) see above list | cc | 0.3-0.6   |

## Part Ib (alternative):

|                                                     |    |           |
|-----------------------------------------------------|----|-----------|
| Elvanol 90-25 (15.0%)                               | g  | 200.0     |
| Potassium bromide (50.0%)                           | cc | 15.0-20.0 |
| Potassium iodide (10.0%)                            | cc | 2.0-8.0   |
| Ampholytes: A-24, 70, 71, 75, 78, 79 or 83 (0.01 M) | cc | 0.5-5.0   |
| Cationics: (0.01 M) see above list                  | cc | 0.0-0.3   |

## Part Ic (alternative):

|                                                     |    |           |
|-----------------------------------------------------|----|-----------|
| Elvanol 90-25 (15.0%)                               | g  | 200.0     |
| Potassium bromide (50.0%)                           | cc | 15.0-20.0 |
| Potassium iodide (10.0%)                            | cc | 2.0-8.0   |
| Ampholytes: A-24, 70, 71, 75, 78, 79 or 83 (0.01 M) | cc | 0.5-1.0   |
| Cationics: (0.01 M) see above list                  | cc | 0.1-0.5   |

## Part II:

|                |    |      |
|----------------|----|------|
| Silver nitrate | g  | 10.0 |
| Water          | cc | 50.0 |

In alternative Part Ia, the poorly peptizing amide containing alpha betaines must be used in combination with the surface-active cationics. In alternative Part Ib, a good or fair peptizing betaine may be used alone, or if

necessary, in combination with small amounts of the cationic components. The ampholytes in alternative Part Ic are intentionally used in a low concentration range in which they will not peptize satisfactorily by themselves, and are brought up to optimum activity by the addition of the cationic materials.

Part II is added to Part Ia, Ib or Ic over a period of 1 to 30 minutes at a temperature of 70° C., and the whole is allowed to digest at 70° C. for 30 minutes. The emulsions are washed by dialysis for 15 hours at 20° C. according to the procedure described above. The following components are added per 100.0 g. of emulsion, and the emulsions are then ripened at 50° C. for 30 minutes:

|                                             |              |
|---------------------------------------------|--------------|
| Sodium thiosulfate (0.001 M)                | 0.5-2.0 cc.  |
| Sodium benzenesulfinate (20.0%)             | 2.0 cc.      |
| Gold solution (prepared as described above) | 0.8 cc.      |
| Sodium carbonate (1.0%)                     | 0.0-2.0 cc.  |
| Potassium iodide (1.0%)                     | 0.5-1.0 cc.  |
| or                                          |              |
| Potassium bromide (1.0%)                    | 1.0-2.0 cc.  |
| and/or                                      |              |
| Stabilizer S-3 (0.01 M)                     | 0.2-1.0 cc.  |
| and/or                                      |              |
| Stabilizer S-27 (0.01 M)                    | 0.2-1.0 cc.  |
| and/or                                      |              |
| Stabilizer S-30 (0.01 M)                    | 0.2-1.0 cc.  |
| and/or                                      |              |
| Stabilizer S-37 (0.01 M)                    | 0.2-1.0 cc.  |
| Prior to coating, there is added:           |              |
| Optical sensitizing dye (0.05%)             | 1.0-10.0 cc. |
| Saponin (8.0%)                              | 1.6 cc.      |
| Water                                       | As required  |

The coated emulsions, when processed as described above, possess photographic characteristics comparable to typical high speed negative emulsions of the gelatin emulsion system such as Ansco Isopan, All Weather Pan, Supreme Pan, Triple S Pan Portrait or Superpan Press Portrait films.

Although I prefer to use polyvinyl alcohol as the synthetic polymeric carrier because of its availability and desirable properties, this invention contemplates the application of other photographic silver halide carrying vehicles which do not possess the natural or inherent sensitizing factors found in gelatin. Examples of such materials are: methyl cellulose, cellulose sulfate, hydroxy ethyl cellulose, carboxy methyl cellulose, gum arabic, gum tragacanth, mesquite gum, gum ghatti, starch, albumin, zein, collodion, polyacrylamide, polyvinylpyrrolidone, and polymers derived from unsaturated materials such as styrene, maleic acid, etc.

This invention has disclosed the preparation and sensitization of silver halide dispersions in synthetic colloid carriers such as polyvinyl alcohol. Nevertheless, it is to be understood that the principles disclosed herein may be also extended to apply to the silver halide-gelatin emulsion systems. In this connection, reference is made to commercially available gelatins which may be unacceptable physically or may be deficient in natural sensitizers or restrainers. Thus, it is contemplated that synthetic additives of the types disclosed herein may find wide application for increasing the silver halide carrying capacity, increasing the degree of peptization and modifying the physical and chemical ripening properties of such gelatins, and for improving generally the sensitometric characteristics of the photographic emulsions prepared therefrom.

## PREPARATION OF COMPOUNDS

Due to the large number of chemical compounds involved, only representative syntheses are presented. Thus, the preparation of a tertiary alkylamine having at least one straight long chain alkyl radical will serve to illustrate the general mode of synthesis of all members of the series. In certain instances, when the compounds are

commercial products, the name and manufacturer or other source is cited. When the compounds are known in the chemical literature, reference is made thereto.

The preparations of the compounds are taken up in the same order as they are listed in Tables I, II and III, above. For the sake of brevity, names or formulae are not given, but the compounds are identified by their C (cationic), A (ampholyte) and S (stabilizer) numbers.

*Cationics (C)*

C-1, which can be any one of several long straight chain primary alkylamines wherein the long chain is an alkyl radical of at least 8 carbon atoms is manufactured by the Armour Chemical Company, Chicago 9, Illinois, under the trade name "Armeens."

C-2, M.P. 41-42° C., was prepared according to the method described in German Patent 657,358.

C-3, a suspension of 66 g. (2.2 moles) of paraformaldehyde in 170.5 g. (4 moles) of formic acid (90% aqueous) was stirred and heated while a hot solution of 213

g. (1 mole) of tetradecylamine ("Armeen 14D," Armour Co.) in 500 ml. of benzene was added at such a rate as to maintain incipient flooding of the reflux condenser. After the completion of the addition, the solution was stirred and boiled for an hour and a half. The solution was cooled, and a solution of 187 g. (2.73 moles) of potassium hydroxide (85% pellets) in 325 ml. of methanol was added with stirring. The mixture was stirred for half an hour, and then the layers were separated. The benzene layer was allowed to remain over sodium hydroxide pellets overnight. The benzene solution was removed by decantation and the solvent was removed by evaporation. Distillation of the residue under reduced pressure gave a yield of 184.7 g. (76.5% of the theoretical amount), B.P. 115-125° C./0.06-0.07 mm., of N,N-dimethyltetradecylamine.

C-4 and C-5 were prepared as above for C-3 except that hexadecyl ("Armeen 16D") and octadecylamine ("Armeen 18D") were used in place of tetradecylamine ("Armeen 14D").

C-6 was obtained from the Rohm and Haas Company, 222 W. Washington Sq., Philadelphia 5, Pa., under the trade name "Opeedma."

C-7 was prepared by combining 2 moles of ethylene diamine with 1 mole of 1,10-dibromodecane as described in Rec. Trav. Chim. 58, 544 (1939).

C-8 was prepared by heating 0.1 mole of 1,10-dibromodecane and 0.3 mole of morpholine in ethanol. The insoluble material was removed by filtration and the filtrate was fractionated in vacuo. The portion distilling at 186-190° C. was collected and purified by dissolution in aqueous acetic acid and precipitation with 10% sodium hydroxide solution.

C-9 was prepared similarly to C-8 except that n-dibutylamine was used in place of morpholine. The boiling point of the product was 109-115° C./15 mm.

C-10 was obtained by heating under reflux 1.2 moles of diethylamine and 0.2 mole of 1,10-dibromodecane in benzene. The insoluble material was removed by filtration and the filtrate was distilled in vacuo. The product, boiling at 142-145° C./1 mm., was collected.

C-11 was prepared by heating  $\alpha$ -aminolauric acid in ethanol saturated with hydrogen chloride. The alcohol was removed by distillation and the residue was crystallized from a mixture of ethanol and petroleum ether. The product melted at 67° C.

C-12 was prepared by dissolving  $\alpha$ -aminolauric acid methyl ester in methanol and saturating the solution with ammonia. After being allowed to stand for 5 days, the solvent and ammonia were removed by distillation and the residue was crystallized from aqueous methanol. The product melted at 90-91° C.

C-13 was prepared by reacting 0.342 mole of methyl N,N-dimethylglycinate with 0.31 mole of hexadecylamine in the presence of 1.0 g. of anhydrous sodium carbonate.

The mixture was then heated for several hours at a maximum pot temperature of 220° C. The cooled residue was poured into water. The water was separated, and the organic layer was distilled in vacuo. The fraction boiling at 165-180° C./0.05-0.09 mm. was collected. M.P. 48-49° C.

C-14 was prepared by first heating 0.5 mole of sodium chloroacetate with 2.4 moles of diethylamine under reflux for several hours. The excess amine was removed under reduced pressure and the residue was then treated with 230 ml. of methanol containing 0.5 mole hexadecylamine. The alcohol was removed by distillation and the residue was heated at 240° C. for three hours. The product was distilled in vacuo and the fraction boiling at 172-175° C./0.05 mm. was collected.

C-15 was prepared by heating 0.3 mole of caprylic acid and 0.33 mole of 3-dimethylaminopropylamine. The reaction time was 30 minutes at 200-230° C. The product was distilled in vacuo and the fraction boiling at 155-156° C./0.6 mm. was collected.

In like manner, cationics C-16, C-17, C-18, C-19 and C-20 were prepared using the appropriate fatty acid or acid halide. The physical constants of these compounds are:

C-16, B.P. 175-178° C./2 mm.

C-17, B.P. 195-204° C./1 mm.

C-18, B.P. 173-178° C./0.09 mm.

C-19, B.P. 194-197° C./0.08 mm.; M.P. 57-58° C.

C-20 could not be distilled and the reaction product was purified by crystallization from acetone; M.P. 62-64° C.

C-21 was prepared from 2 moles of benzylamine and 1 mole of n-tetradecyl bromide according to the method described in J. Chem. Soc., 401 (1942).

C-22 was prepared by heating 0.2 mole of sebacyl chloride and 0.4 mole of 3-dimethylaminopropylamine in 100 ml. of dry benzene at reflux temperature for 2 hours. The benzene and excess amine were removed by filtration and the residue was crystallized from benzene; M.P. 100-102° C.

C-23 was prepared according to the method given for C-15, but using stearoyl chloride and 2-diethylaminoethylamine. The product melted at 61-62° C.

C-24 was obtained by heating 0.05 mole of 6-aminoquinoline with 0.05 mole of myristoyl halide in 25 ml. of pyridine for 2 hours on a steam bath. The mixture was poured into water and the solid residue was crystallized from a mixture of ethanol and petroleum ether; M.P. 90-91° C.

C-25 was prepared according to the method given above for C-24 but using 2-aminopyridine in lieu of 6-aminoquinoline.

C-26 was prepared by the polymerization of 4-vinyl pyridine using ammonium persulfate as the catalyst.

C-27 was prepared by heating under reflux a mixture of 0.1 mole of octylamine and 0.1 mole of S-methyl isothiouronium p-toluene sulfonate in 25 ml. of ethanol for 6 hours. The product which was crystallized from acetone melted at 82-83° C.

The following compounds were prepared in the manner given above for C-27 but substituting the appropriate long chain amine.

C-28, M.P. 94-95° C.

C-29, M.P. 103° C.

C-30, M.P. 76-80° C.

C-31, M.P. 79-85° C.

C-32, M.P. 87-91° C.

C-33, M.P. 88-89° C.

C-34 was prepared by heating under reflux 0.67 mole of dodecylamine p-toluenesulfonate and 0.66 mole of di-cyandiamide in 50 ml. of dimethylformamide for 3.5 hours. 12.5 grams of copper sulfate.5H<sub>2</sub>O in 50 ml. of dimethylformamide was then added and the pink copper complex of C-34, which precipitated, was removed

by filtration. The complex was broken up by heating in the presence of glacial acetic acid and p-toluenesulfonic acid and the copper-free product was crystallized from methanol; M.P. 217-218° C.

C-35 was obtained as above for C-34 except that hexadecylamine was substituted for dodecylamine; M.P. 208-210° C.

C-36 was prepared from 4-decoxyaniline and dicyandiamide according to the procedure described in United States Patent 2,704,710.

C-37 was prepared by first heating 15 g. of polyoxyethylene and 0.5 mole of aniline in 300 ml. of 95% ethanol. A condensation product was obtained which melted at 137-138° C. and which was presumably the polymeric anil. This material was treated with 0.2 mole of dicyandiamide in 100 ml. of water and 16.4 ml. of concentrated hydrochloric acid and the whole was boiled for 30 minutes. Upon treatment with mineral alkali, a solid was obtained which was dissolved in acetic acid and precipitated by means of acetone.

C-38 and other tertiary amine oxides are described in United States Patents 2,169,976; 2,185,163 and 2,159,967.

C-39 was prepared by heating under reflux 0.03 mole of dimethylhexadecylamine and 0.033 mole of methyl p-toluenesulfonate in 100.0 cc. of acetone for 2 hours. The mixture was cooled, diluted with ether and the solid material was removed by filtration. The crude product which was crystallized from ethanol melted at 223-229° C./dec.

The following compounds, C-40 to C-67 inclusive were purchased on the chemical market or were prepared according to the method for C-39. For the sake of brevity, only the quaternizing agent is named since the structure of the tertiary amine, prior to quaternization, is apparent by reference to the various structures.

C-40 is described in United States Patent 2,075,958.

C-41, from dibutyloctadecylamine and methyl p-toluenesulfonate, M.P. 69-70° C.

C-42 is prepared as described in J.A.C.S., 68, 755 (1946).

C-43 was prepared from the tertiary amine and ethyl bromoacetate; M.P. 54-56° C.

C-44 was obtained from the Rohm & Haas Company under the trade name "Hyamine 1622."

C-45 was prepared from the long chain alkyl amido tertiary amine and methyl-p-toluenesulfonate; M.P. 132-134° C.

C-46 was prepared from the long chain alkyl amido tertiary amine and methyl-p-toluenesulfonate; M.P. 89-91° C.

C-47 was prepared from the long chain alkyl amido tertiary amine and methyl-p-toluenesulfonate; M.P. 86° C.

C-48 was prepared from the long chain alkyl amido tertiary amine and methyl-p-toluenesulfonate; M.P. 110-111° C.

C-49 was prepared from the long chain alkyl amido tertiary amine and methyl-p-toluenesulfonate; M.P. 111-112° C.

C-50 was prepared from the long chain alkyl amido tertiary amine and chloroacetamide; M.P. 89-90° C.

C-51 was prepared from the long chain alkyl amido tertiary amine and methyl-p-toluenesulfonate; M.P. 105-107° C.

C-52 was prepared from the long chain alkyl amido tertiary amine and ethyl bromoacetate; M.P. 62-64° C.

C-53 was prepared from the long chain alkyl amido tertiary amine and ethyl  $\gamma$ -bromobutyrate; M.P. 62-65° C.

In preparing the aforesaid compounds numbered C-45 through and including C-53, except C-51, the long chain

alkyl amido tertiary amines employed therein were prepared from the corresponding long chain fatty acid and 3-dimethylaminopropylamine.

The intermediate for C-51 was prepared by first combining stearoyl chloride with glycine to produce N-stearoyl glycine, M.P. 120-122° C. This product was converted to its methyl ester by heating with a solution of hydrogen chloride dissolved in methyl alcohol. The ester, melting at 78° C., was then treated with 3-dimethylaminopropylamine to yield the N(3-dimethylaminopropyl)-2-stearamidoacetamide, melting at 97-99° C.

C-54 was prepared from the long chain alkenyl succinimido tertiary amine and chloroacetamide.

C-55 was prepared from the long chain alkenyl succinimido tertiary amine and ethyl bromide; M.P. 170-172° C.

C-56 was prepared from the succinimido tertiary amine and bromo N-octadecylacetamide; M.P. 187-188° C.

C-57 was prepared from succinimido tertiary amine and hexadecyl bromide; M.P. 160-162° C.

C-58 was prepared from the acetamido tertiary amine and hexadecyl-p-tolene sulfonate; M.P. 134-135° C.

C-59 was prepared from the long chain alkenyl succinimido tertiary amine and phenacyl bromide.

C-60 was prepared from the N-long chain alkyl- $\alpha$ -dimethylamino-acetamide methyl p-tolene sulfonate; M.P. 112-113° C.

C-61 was prepared from the N-long chain alkyl- $\alpha$ -dimethylaminoacetamide and benzyl bromide; M.P. 140-141° C.

C-62 was prepared from the N-long chain alkyl- $\alpha$ -dimethylaminoacetamide and phenacyl bromide; M.P. 142-144° C.

C-63 was prepared from the N-long chain alkyl- $\alpha$ -diethylaminoacetamido and ethyl bromoacetate; M.P. 71-73° C.

C-64 was prepared from the N-long chain alkyl- $\alpha$ -diethylaminoacetamide and ethyl- $\gamma$ -bromo n-butyrate; M.P. 37-38° C.

C-65 was prepared from the long chain alkoxy benzamido tertiary amine and methyl p-toluenesulfonate; M.P. 126-127° C.

C-66 was prepared from the long chain alkyl amido benzamido tertiary amine and methyl p-toluenesulfonate; M.P. 158° C.

C-67 was prepared from the long chain alkyl amido benzamido tertiary amine and methyl p-toluenesulfonate; M.P. 155° C.

In the above compounds numbered from C-54 through and including C-57, the succinimido tertiary amines were prepared from the corresponding succinic anhydride and 3-dimethylaminopropylamine. The acetamido tertiary amine for C-58 was prepared from acetic acid or acid anhydride and 3-dimethylaminopropylamine.

For compounds C-60 through C-64, the N-long chain alkyl- $\alpha$ -dimethylamino and diethylaminoacetamides were prepared from the corresponding long chain alkyl amines and the appropriate N,N-dimethyl or N,N-diethyl-glycine ester.

The long chain alkoxy benzamido tertiary amine required for C-65 was prepared from p-hexadecoxy benzoic acid and 3-dimethylaminopropylamine.

The long chain acylamido benzamide tertiary amine intermediates required in preparing C-66 and C-67 were prepared from p- and m-palmitamidobenzoic acid and 3-dimethylaminopropylamine.

Compounds C-68 through and including C-79 are quaternary salts of heterocyclic bases and, in general, can be prepared by heating equimolar quantities of a desired heterocyclic base and the appropriate quaternizing agent. Thus, C-68 was prepared by heating 1 mole of hexadecyl bromide and 1 mole of pyridine. The resulting quaternary salt melted at 58-59° C.

C-69 was prepared according to C-68, using octadecyl

- p-toluenesulfonate and pyridine, melted at 129-130° C. C-70 was prepared from  $\alpha$ -bromolauramide and pyridine; M.P. 147-148° C.
- C-71 was prepared from N-octylnicotinamide and methyl p-toluenesulfonate; M.P. 104° C.
- C-72 was prepared from N-decylnicotinamide and methyl p-toluenesulfonate; M.P. 112-113° C.
- C-73 was prepared from N-dodecylnicotinamide and methyl p-toluenesulfonate; M.P. 116° C.
- C-74 was prepared from N-hexadecylnicotinamide and methyl p-toluenesulfonate; M.P. 110-111° C.
- C-75, M.P. 95-97° C., was prepared from N-hexadecyl-nicotinamide and benzylbromide.
- C-76, M.P. 106-107° C., was prepared from N-hexadecylnicotinamide and ethyl bromoacetate.
- C-77, M.P. 101-102° C., from nicotinic acid ethyl ester and hexadecylbromide.
- C-78 was prepared from 4-polyvinylpyridine and butyl bromide.
- C-79, M.P. 137-138° C., was obtained from 2-methyl-benzothiazole and octadecyl p-toluenesulfonate.
- C-80, M.P. 156-161° C., was obtained by heating 1 mole of unsym. dimethyl hydrazine with  $\frac{1}{2}$  mole of dodecylbromide in ethanol.
- C-81, M.P. 178-180° C., was obtained from unsym. dimethyl hydrazine and hexadecyl p-toluenesulfonate.
- C-82, M.P. 177-179° C., was obtained from unsym. dimethyl hydrazine and octadecyl p-toluenesulfonate.
- C-83, M.P. 75-76° C., was prepared from C-81 and acetic anhydride by heating on the steam bath for 15 hours.
- C-84 was prepared by heating 0.05 mole of palmitic acid dimethyl hydrazide and 0.1 mole of methyl p-toluenesulfonate for 5 hours on a steam bath. The reaction mixture was dissolved in acetone and the product was precipitated with dry ether; M.P. 100-102° C.
- C-85, M.P. 113-114° C., was prepared as described above for C-84 except that stearic acid unsym. dimethyl hydrazide was used in place of the palmitic acid hydrazide.
- C-86, M.P. 152-154° C., was prepared from palmitic acid dimethyl hydrazide and ethyl bromoacetate.
- C-87 was prepared from p-palmitamidobenzoic acid unsym. dimethylhydrazide; M.P. 156-159° C.
- C-88, M.P. 129-130° C., was prepared from p-hexadecoxybenzoic acid unsym. dimethyl hydrazide and methyl p-toluenesulfonate.
- C-89 was prepared from .01 mole of hexadecyldimethylamine (C-4) and 0.01 mole of 2-chlorobenzothiazole by heating on a steam bath for 7 hours. The reaction mixture was triturated with ether, cooled, and the solid was filtered off. Purification was effected by dissolving the crude product in hot acetone followed by precipitation with dry ether. The melting point of purified quaternary salt was 225-226° C.
- C-90 was prepared from 0.01 mole of N-(3-dimethylaminopropyl) stearamide described above and 0.02 mole of 2-chlorobenzothiazole by heating on a steam bath for 12 hours.
- C-91, M.P. 228-230° C., was obtained by heating a mixture of 0.02 mole of 2-chloroquinoline and 0.01 mole of hexadecyldimethylamine.
- C-92 was prepared by heating on a steam bath for 1 hour, a mixture of 0.005 mole of unsym. N,N-dimethylhexadecanesulfonhydrazide and 0.01 mole of methyl p-toluenesulfonate. The reaction mixture was triturated with dry ether, after which it was purified by dissolving in hot acetone followed by precipitation with dry ether. The purified, light cream colored product melted at 105-106° C. The prerequisite sulfohydrazide was prepared from 0.02 mole of 1-hexadecane sulfonyl chloride and 0.033 mole of unsym. dimethyl hydrazine in the presence of aqueous sodium carbonate. The melting point of the resulting unsym. N,N-dimethyl-hexadecanesulfonhydrazide was 66-67° C.
- C-93, M.P. 70-71° C., was prepared by the alkylation

- of 0.04 mole of tetradecylethylsulfide with 0.04 mole of methyl iodide in the presence of 50 ml. of methanol. The reaction was carried out by heating the above ingredients for 6 hours on a steam bath. Purification was effected by crystallization from a mixture of 95% ethanol and ether. This method is the general applicability for preparing alkyl sulfonium halides.
- C-94, M.P. 125° C., was prepared by the quaternization of N-(3-dimethylaminopropyl) hexadecanesulfonamide with methyl p-toluenesulfonate. The prerequisite sulfonamide was prepared by heating hexadecanesulfonyl chloride, M.P. 49-50° C., with 3-dimethylaminopropylamine in benzene solution. The intermediate, after recrystallization from petroleum ether, melted at 68-69° C.
- C-95, M.P. 131-132° C., was prepared from N(3-dimethylaminopropyl) - 4 - lauramidobenzenesulfonamide and methyl p-toluenesulfonate. The prerequisite sulfonamide was prepared by heating 4-lauramidebenzenesulfonyl chloride, M.P. 67-69° C., with 3-dimethylaminopropylamine in benzene solution. The intermediate, after recrystallization from a mixture of benzene and petroleum ether, melted at 77-78° C.
- Ampholytes (A)*
- As with the cationics, detailed preparations are given only for representative compounds. Individual ampholytes (A) that fall under a general synthesis are thus referred back to the detailed method of preparation. In some instances, the source of the components is the commercial chemical market in which case reference is made as to the manufacturer.
- The compounds beginning with A-1 and concluding with A-21 are various aminocarboxylic acids, with the exception of A-8 which is a taurine derivative, and were prepared by reacting an amino containing component with the appropriate halogen containing component.
- A-1 was obtained by heating 0.1 mole of dodecylamine with 0.1 mole of sodium bromoacetate in 20 ml. of 50% (vol.) ethanol. After 8 hours, the solvent was removed by distillation in vacuo, and the residue taken up in methanol to which was added an equal volume of acetone. After cooling, the solid material was removed by filtration and was crystallized from methanol-acetone.
- A-2 was prepared according to the method above for A-1 but using hexadecylamine instead of dodecylamine.
- A-3 was prepared as above for A-1 but using octadecylamine for dodecylamine.
- A-4 is a product sold by the B. F. Goodrich Chemical Company, 500 S. Main Street, Akron, Ohio.
- A-5 was prepared similarly to A-1 except that hexadecylamine and sodium bromopropionate was used.
- A-6 was prepared by heating under reflux 0.038 mole of N-hexadecyl-2-pyrrolidone with a solution of 20 cc. of concentrated hydrobromic acid in 50 cc. of water for 26 hours. The reaction mixture was cooled, and a solid was removed by filtration and dried in vacuo. The product was purified by crystallization from a mixture (1:10 by volume) of ethanol and petroleum ether.
- A-7 was prepared by heating 0.03 mole of  $\epsilon$ -aminocaproic acid hydrobromide, 0.03 mole of tetradecyl bromide, 0.06 mole of sodium hydroxide dissolved in 5 ml. of water, and 25 ml. of ethanol under reflux for 4 hours. After removal of the solvent in vacuo, the residue was crystallized from a mixture of equal volumes of methanol and acetone.
- A-8 was prepared from dodecylamine and sodium bromomethane sulfonate according to the procedure described in United States Patent 2,652,328.
- A-9 was prepared from molar proportions of sodium chloroacetate and methyl octadecylamine by heating for 11 hours on a steam bath using toluene as the solvent. The crude product was purified by crystallization from methanol-acetone.

A-10 was prepared from  $\alpha$ -bromo lauric acid and concentrated ammonium hydroxide containing a trace of ammonium carbonate by heating at 58° C. for 3 hours. The white solid, after crystallization from acetic acid, melted at 263° C.

A-11 was obtained by heating 0.1 mole unit of 1-vinyl-2-pyrrolidone polymer with a solution of 90 ml. of 40% hydrobromic acid and 120 cc. of water under reflux for 20 hours. After evaporation in vacuo, the residue was dissolved in ethanol and precipitated with acetone.

A-12 was obtained by the copolymerization of 2-vinylpyridine and acrylic acid.

A-13 resulted by heating 0.2 mole of sodium bromoacetate with 0.1 mole of hexadecylamine in aqueous ethanol under reflux. The ethanol was evaporated in vacuo and the residue was crystallized from aqueous ethanol and acetone. The purified product decomposed at 160° C.

A-14 was obtained by heating 0.02 mole of sodium bromoacetate and 0.02 mole of  $\alpha$ -amino lauric acid in aqueous methanol, under reflux. The solvent was removed in vacuo and the residue was purified by crystallization from methanolacetone.

A-15 was obtained by treating 0.3 mole of sodium bromoacetate and 0.1 mole of N-dodecylethylenediamine in aqueous methanol.

A-16 was prepared by heating 0.1 mole of  $\alpha$ -bromo lauric acid and 0.3 mole of ethanolamine in aqueous methanol for 5 hours.

A-17, M.P. 174-175° C., was prepared as described in J. Chem. Soc., 99, 572 (1911).

A-18,  $\epsilon$ -benzoylaminoo- $\alpha$ -bromocaproic acid, which had been prepared according to the method described in "Organic Synthesis," Coll. Vol. II, page 74, was condensed with hexadecylamine to produce  $\epsilon$ -benzoylaminoo- $\alpha$ -hexadecylamino caproic acid. The above intermediate was hydrolyzed with 40.0% hydrobromic acid to yield the desired  $\epsilon$ -amino- $\alpha$ -hexadecylamino caproic acid (A-18).

A-19, M.P. 108° C., was prepared as described in J. Chem. Soc., 99, 1584 (1911).

A-20 was prepared according to the method disclosed in United States Patents 2,320,232 and 2,312,967.

A-21 resulted from the alkaline hydrolysis of N-(3-dimethylaminopropyl)octadecenylsuccinimide with sodium hydroxide in methanol.

Ampholytes A-22 through and including A-93 belong to that class of chemical compounds known in the art as betaines. Such compounds can be prepared by heating a tertiary amine with a halo aliphatic acid in the presence of an alkali such as sodium hydroxide which forms the betaine plus sodium halide. Such a method, however, usually leads to rather impure products since it is difficult to separate the water-soluble betaine from the inorganic salts. I prefer to prepare the betaines used herein by the method described in copending application, Serial Number 642,384, filed February 26, 1957, by Robert M. Lindquist, which comprises treatment of the product produced by reacting a tertiary amine with a halo carboxylic ester with a highly basic ion exchange resin such as "Amberlite IRA-400," wherein the resin cleaves the quaternary ester and retains the halide ions leaving a solution of the desired betaine free from inorganic salts.

Many of the various complex tertiary amines used in preparing the aforementioned "Betaines" have already been described under preparation of the "Cationics" (C).

The following typical preparations illustrate the general synthetic methods which were employed:

A-24, solutions of 30.6 g. (0.22 mole) of bromacetic acid in 200.0 ml. of methanol, 59.5 g. (0.2 mole) of dimethyloctadecylamine (C-5) in methanol and 9.1 g. (0.22 mole) of sodium hydroxide (97.0% pellets) in 200.0 ml. of methanol were combined and the whole was heated under reflux for 2 hours. The methanol

was removed by distillation under vacuum and the residue was triturated with boiling acetone. The product was dissolved in 175.0 ml. of hot isopropyl alcohol and isopropyl alcohol insoluble salts were removed by filtration. The filtrate was cooled, diluted with acetone and the betaine, which separated, was removed by filtration and washed with acetone. The yield of product was 69.0 g.

A-43, solutions of 30.6 g. (0.22 mole) of bromacetic acid in 200.0 ml. of methanol, 73.8 g. (0.2 mole) of N-(3-dimethylaminopropyl)stearamide (C-20) in methanol and 9.1 g. (0.22 mole) of sodium hydroxide (97% pellets) in 200.0 ml. of methanol were combined and the whole was heated under reflux for 2 hours. The methanol was then removed by distillation under vacuum. The residue was heated with 750.0 ml. of isopropyl alcohol and the insoluble material was removed by filtration. The filtrate was cooled and the solid, which separated, was removed by filtration and was washed with several 100.0 ml. portions of cold isopropyl alcohol. The betaine, which was purified by recrystallization from 900.0 ml. of isopropyl alcohol, weighed 75.0 g.

A-49 was prepared in a manner analogous to A-43, using 2.3 g. of bromacetic acid, 6.38 g. of N-(3-dimethylaminopropyl)-2-stearamidoacetamide and 0.68 g. of sodium hydroxide in methanol.

A-71 was prepared in a manner analogous to A-24, using 8.63 g. of N-bromacetyl glycine, 11.9 g. of dimethyloctadecylamine and 1.82 g. of sodium hydroxide in methanol.

A-75 was prepared in a manner analogous to A-24 using 43.1 g. of N-bromacetyl glycine, 73.6 g. of N-(3-dimethylaminopropyl)stearamide and 9.1 g. of sodium hydroxide in 500.0 cc. of methanol. The yield of betaine was 103.0 g.

A-78, N-(3-dimethylaminopropyl)succinimide was prepared from 50.0 g. of succinic anhydride and 56.0 g. of 3-dimethylaminopropylamine by heating the components at 200-220° C. The product was distilled and the fraction boiling at 108-110° C./0.07 mm. was collected.

A solution of 7.35 g. of N-(3-dimethylaminopropyl)succinimide, 12.2 g. of hexadecyl bromide in 100.0 cc. of acetone was heated under reflux for 15 hours. The solution was cooled and the dimethylhexadecyl(3-succinimidopropyl)ammonium bromide, which separated, was removed by filtration. After recrystallization from acetone, the product melted at 160-162° C.

The above quaternary salt (9.78 g.) and 0.83 g. of sodium hydroxide in 25.0 ml. of methanol was heated under reflux for 8 hours. The methanol was removed under vacuum and the residue was digested with boiling isopropyl alcohol. The insoluble salts were removed by filtration and the filtrate was evaporated to dryness. The residual oil was triturated with several portions of boiling acetone, yielding 8.8 g. of product A-78.

A-83 was synthesized using the general procedure described for A-78 in which octadecenylsuccinic anhydride was used in place of succinic anhydride and quaternization was carried out with ethyl bromide instead of hexadecyl bromide.

A-94, hexadecanesulfonyl chloride was prepared by heating a mixture of 64.0 g. of sodium hexadecanesulfonate, 40.5 g. of phosphorous pentachloride and 100.0 ml. of phosphorous oxychloride under reflux for 3 hours. The phosphorous oxychloride was removed under reduced pressure and the residue was treated with hot petroleum ether. The solid, which was removed by filtration, weighed 18.0 g. and melted at 4950° C.

A solution of 24.5 g. of the above hexadecanesulfonyl chloride and 30.9 g. of 3-dimethylaminopropylamine in 400.0 ml. of dry benzene was heated on a steam bath for 2 hours. The mixture was cooled to room temperature

and was shaken with a dilute aqueous solution of sodium bicarbonate. The benzene layer was separated and the benzene was removed by distillation. The N-(3-dimethylaminopropyl)hexadecanesulfonamide, after crystallization from high boiling petroleum ether, weighed 18.0 g. and melted at 68-69° C.

N-(3-dimethylaminopropyl)hexadecanesulfonamide was condensed with bromacetic acid in a manner analogous to that previously described for the preparation of the carboxamide containing betaines. Product A-94 melted at 113-114° C.

A-95 was prepared from equimolar quantities of tetradecyl ethyl sulfide and chloroacetic acid.

A-96, M. P. 200-205° C., was prepared by heating 1 equivalent of arginine monohydrochloride and 1 equivalent of lauroyl chloride in the presence of 2 equivalents of sodium hydroxide.

A-97 was prepared by heating hexadecylmethyl-2-bromethylammonium bromide with an excess of sodium sulfite in aqueous media.

A-98 was prepared by heating hexadecylmethyl-2-bromethylammonium bromide and sodium thiosulfate in ethanol.

A-99 was prepared from dodecyltaurine (A-8) and cyanamide in ethanol according to the procedure described in United States Patent 2,652,328.

A-100 was prepared from N-(3-dimethylaminopropyl)-4-lauramido benzenesulfonamide and bromacetic acid in a manner analogous to that previously described for the carboxamide containing betaines. Product A-100 melted at 210-212° C.

A-101 and A-102 were purchased from the Miranol Chemical Company, Inc., 277 Coit Street, Irvington, N.J., under the trade names, "Miranol C2M" and "Miranol OM," respectively.

#### Antifoggants and Stabilizers (S)

S-1 through S-8 are stabilizers well-known to the photographic art and reference is made to the chemical literature for their method of preparation.

S-9 was prepared according to the method of Jones, J.A.C.S., 71, 4000 (1943).

S-10 was prepared by the oxidation of iminothiourazole in alkaline solution using potassium persulfate as the oxidation agent.

S-11 was prepared by heating a mixture of o-phenylenediamine and lauric acid at 150 to 200° C. After recrystallization from ethanol, the pure product melted at 107° C.

S-12 was prepared by combining equimolar quantities, at room temperature, of 2-aminobenzimidazole and tetradecanoyl chloride in acetone solution in the presence of excess triethylamine.

S-13 was prepared by heating equimolar proportions of 1-histidine monohydrochloride and tetradecanoyl chloride in aqueous ether solution using triethylamine as the condensing agent. The crude product, after recrystallization from a mixture of water and methanol, melted at 112° C.

S-14 was prepared by heating equimolar proportions of histidine methyl ester dihydrochloride with tetradecanoyl chloride in chloroform in the presence of triethylamine. After crystallization from ethyl acetate, the purified product melted at 118-119° C.

S-15 was prepared by heating guanine with an excess of tetradecanoyl chloride in the presence of dry pyridine. The product was purified by crystallization from ethanol.

S-16 was prepared according to a method disclosed in Fiat Report #943, page 80.

S-17 was prepared by acylating 5-aminotetrazole with an excess of decanoyl chloride in a mixture of pyridine and chloroform. After crystallization from 95% ethanol, the purified product melted at 224-225° C.

S-18 was prepared by heating 5-aminotetrazole with a

slight excess of tetradecanoyl chloride in a solution composed of a mixture of dry pyridine and dry chloroform. After crystallization from absolute ethanol, the purified product melted at 220° C.

S-19 was prepared according to the method described in J.A.C.S. 49, 2064 (1927).

S-20 was prepared by heating under reflux equimolar quantities of tetradecyl bromide and thiourea in 95% alcohol. The resulting hydrobromide salt was recrystallized from water containing excess hydrobromic acid.

S-21 was prepared by heating equimolar proportions of dodecylamine and thioglycolic acid and dry benzene. The crude product was purified by crystallization from ethanol.

S-22 was prepared in manner similar to S-21, using hexadecylamine in place of dodecylamine.

S-23 was prepared in a manner similar to S-21, using octadecylamine in place of dodecylamine.

S-24 was purchased by the Connecticut Hard Rubber Company.

S-25 was prepared from equimolar quantities of sodium thiosulfate and  $\alpha$ -bromo-N-octadecyl acetamide. The crude product, after crystallization from absolute ethanol, melted at 175-180° C. (dec.).

S-26 was prepared by acylating the amino group on 6-amino-2-mercaptopbenzothiazole with a slight excess of decanoyl chloride in aqueous sodium hydroxide solution. The purified product, after crystallization from chlorobenzene, melted at 165-166° C.

S-27 was prepared by acylating 6-amino-2-mercaptopbenzothiazole with a slight excess of lauroyl chloride in the presence of aqueous sodium hydroxide solution. The crude product, after crystallization from chlorobenzene, melted at 171-172° C.

S-28 was prepared analogously to S-27 except that octadecoyl chloride was used in place of lauroyl chloride. S-29 was obtained by the acylation of 5-amino-2-mercaptopbenzimidazole with a slight excess of decanoyl chloride. After crystallization from methanol, the product melted at 257-61° C.

S-30 was prepared analogously to S-29, using lauroyl chloride in place of decanoyl chloride; M.P. 266-267° C.

S-31 was prepared by heating equivalent amounts of octadecenylsuccinic anhydride and 6-amino-2-mercaptopbenzothiazole in glacial acetic acid.

S-32 was prepared by heating under reflux equimolar proportions of 2-chloro-5-lauramido quinoline with thiourea in absolute ethanol. The melting point of the yellow crystalline product was 225-227° C.

S-33 was prepared according to the procedure outlined in S-32 except in this case the isomeric 2-chloro-8-lauramido quinoline was employed. The melting point of the product was 141-143° C.

S-34 was prepared by heating under reflux equivalent amounts of 1-chloro-5-lauramidoisoquinoline and thiourea in ethanol followed by treatment with potassium hydroxide. The product melted at 218-19° C. (dec.).

S-35 was prepared by heating ethyl tetradecanoyl acetate with an excess of thiourea in absolute ethanol containing an excess of sodium ethylate. The product, after recrystallization from benzene, melted at 145° C.

S-36 was prepared by treating 1-cystine with an excess of caprylyl chloride in the presence of n-sodium hydroxide solution. The crude product, after crystallization from a mixture of low boiling petroleum ether and ethyl acetate, melted at 99-100° C.

S-37 was prepared by treating 1-cystine with an excess of lauroyl chloride in the presence of sodium hydroxide solution. The crude product was obtained by acidification of the reaction mixture. After recrystallization from a mixture of alcohol, ether, and petroleum ether, the melting point of the purified product was 112-113° C.

S-38 was prepared according to S-37 but using stearoyl chloride in lieu of lauroyl chloride.

S-39 was prepared by acylating cystine diethyl ester with 2 moles of lauroyl chloride in dry benzene using pyridine as a basic condensing agent. The crude product, after crystallization from absolute alcohol, melted at 97-98° C.

S-40 was prepared according to the procedure described in Am. Soc. 36, 1266 (1914).

S-41 was prepared by heating hexadecyldimethylamine with a slight excess of p-( $\beta$ -bromoethoxy)phenol in absolute alcohol. The crude product was purified by crystallization from acetone.

S-42 was prepared by heating equimolar proportions of 2-bromoethyl, hexadecyl, dimethylammonium bromide and thiourea in absolute alcohol. The reaction mixture was treated with 48% HBr. The crude product was purified by crystallization from a mixture of alcohol and acetone.

S-43 was prepared by heating equimolar amounts of 2-chloromethylbenzimidazole and hexadecyldimethylamine in ethanol. The product was purified by crystallization from acetone.

S-44 was prepared by heating under reflux equimolar proportions of 2-chloromethyl-5-nitrobenzimidazole and hexadecyldimethylamine in absolute alcohol. After crystallization from absolute ethanol, the purified material melted at 196-197° C.

S-45 was prepared by heating under reflux equimolar proportions of 2-bromo acetamido thiazole and hexadecyldimethylamine in absolute methanol.

S-46 was prepared by heating an excess of 5-chloroacetamido tetrazole with hexadecyldimethylamine in isopropyl alcohol. The product was purified by crystallization from acetone.

S-47 was prepared by heating under reflux equimolar proportions of 3-bromo acetamido-1,2,4-triazole and hexadecyldimethylamine in acetone. The crude product, after recrystallization from acetone, melted at 165° C.

S-48 was prepared by heating under reflux 1 equivalent of 4-(5) chloro methyl imidazole hydrochloride with 2 equivalents of hexadecyldimethylamine in absolute ethanol. After removal of the solvent, the product was dissolved in absolute ethanol containing dissolved hydrogen chloride and was precipitated with ether. The purified product melted at 195° C.

S-49 was prepared by heating 1 equivalent of 2-bromo acetamidobenzothiazole with 1 equivalent of hexadecyldimethylamine in absolute ethanol. After evaporation of the solvent, the residue was crystallized from a mixture of acetone and ethanol.

S-50 was prepared by heating under reflux 1 equivalent of  $\alpha$ -bromo myristic acid in an aqueous solution containing 3 equivalents of potassium hydroxide. The resulting crude hydroxy myristic acid was purified by crystallization from a mixture of chloroform and petroleum ether. The purified product melted at 79-80° C.

S-51 was prepared by acylating 4-amino-2-hydroxybenzoic acid with a slight excess of tetradecanoyl chloride in dry benzene. The crude product, after removal of the solvent, was purified by crystallization from 95.0% ethanol. The melting point of the purified product was 138° C.

S-52 was prepared by acylating 5-amino-2-hydroxybenzoic acid with an excess of tetradecanoyl in dry benzene. After removal of the solvent, the crude product was crystallized from ethyl acetate.

S-53 was prepared by sulfonating myristyl alcohol with chloro sulfonic acid in glacial acetic acid at a temperature of 0 to 10° C.

S-54 was prepared according to the method disclosed in S-53 except that octadecyl alcohol was used in place of myristyl alcohol.

I claim:

1. A photographic polyvinyl alcohol light-sensitive

silver halide emulsion produced by precipitating and ripening the silver halide grains in polyvinyl alcohol containing a sensitizing quantity of at least two surface active agents, both having an aliphatic chain of from 8 to 18 carbon atoms, one of said surface active agents being selected from the class consisting of cationic surface active agents having a functional grouping of the class consisting of primary amino ( $-\text{NH}_2$ ), secondary amino ( $>\text{NH}$ ), tertiary amino



quaternary ammonium



hydrazino ( $-\text{NH}-\text{NH}_2$ ), azonium



guanyl



guanido



biguanido



amino oxide



ternary sulfonium



and quaternary phosphonium



the other of said surface active agents being selected from the class of ampholytic surface active agents having a functional grouping selected from the class consisting of primary amino ( $-\text{NH}_2$ ), secondary amino ( $>\text{NH}$ ), tertiary amino



quaternary ammonium



hydrazino ( $-\text{NH}-\text{NH}_2$ ), azonium



guanyl



guanido



biguanido



75

amino oxide



ternary sulfonium



and quaternary phosphonium



the said amphotolytic surface active agent having an additional grouping selected from the class consisting of carboxylic acid ( $-\text{COOH}$ ), sulfonic acid ( $-\text{SO}_3\text{H}$ ), sulfinic acid ( $-\text{SO}_2\text{H}$ ), sulfuric ester ( $-\text{OSO}_3\text{H}$ ), phosphonic acid ( $-\text{PO}_3\text{H}_2$ ), phosphonous acid ( $-\text{PO}_2\text{H}_2$ ), phosphoric monoester ( $-\text{OPO}_3\text{H}_2$ ), phosphoric diester

mercapto ( $-\text{SH}$ ), and phenolic hydroxy ( $-\text{OH}$ ).

2. A process of preparing a photographic polyvinyl alcohol light-sensitive silver halide emulsion which includes precipitating and ripening the silver halide grains in a polyvinyl alcohol containing a sensitizing quantity of at least two surface active agents, both having an aliphatic chain of from 8 to 18 carbon atoms, one of said surface active agents being selected from the class consisting of a cationic surface active agent having a functional grouping of the class consisting of primary amino ( $-\text{NH}_2$ ), secondary amino ( $>\text{NH}$ ), tertiary amino



quaternary ammonium

hydrazino ( $-\text{NH}-\text{NH}_2$ ), azonium

guanyl



guanido



biguanido



amino oxide



ternary sulfonium



and quaternary phosphonium



the other of said surface active agents being selected from the class of amphotolytic surface active agents having a functional grouping selected from the class consisting

primary amino ( $-\text{NH}_2$ ), secondary amino ( $>\text{NH}$ ), tertiary amino



5 quaternary ammonium

10 hydrazino ( $-\text{NH}-\text{NH}_2$ ), azonium

guanyl



guanido



20 biguanido



amino oxide



30 ternary sulfonium



35 and quaternary phosphonium



40 said amphotolytic surface active agent having an additional grouping selected from the class consisting of carboxylic acid ( $-\text{COOH}$ ), sulfonic acid ( $-\text{SO}_3\text{H}$ ), sulfinic acid ( $-\text{SO}_2\text{H}$ ), sulfuric ester ( $-\text{OSO}_3\text{H}$ ), phosphoric acid ( $-\text{PO}_3\text{H}_2$ ), phosphonous acid ( $-\text{PO}_2\text{H}_2$ ), phosphoric monoester ( $-\text{OPO}_3\text{H}_2$ ), phosphoric diester

45

50 mercapo ( $-\text{SH}$ ), and phenolic hydroxy ( $-\text{OH}$ ).

3. A photographic light-sensitive polyvinyl alcohol silver halide emulsion as defined by claim 1, wherein said amphotolytic surface active agent is an amino-carboxylic acid having an aliphatic chain of at least 8 carbon atoms.

55 4. A light-sensitive photographic polyvinyl alcohol silver halide emulsion as defined by claim 1, wherein said cationic surface active agent is a guanidine having an aliphatic chain of from 8 to 18 carbon atoms.

5. A light-sensitive photographic polyvinyl alcohol silver halide emulsion as defined by claim 1, wherein said amphotolytic surface active agent is a betaine having an aliphatic chain of from 8 to 18 carbon atoms.

6. A process of preparing a photographic polyvinyl alcohol light-sensitive silver halide emulsion as defined by claim 2, wherein said amphotolytic surface active agent is an amino-carboxylic acid having an aliphatic chain of at least 8 carbon atoms.

7. A process of preparing a photographic polyvinyl alcohol light-sensitive silver halide emulsion as defined by claim 2, wherein said cationic surface active agent is a guanidine having an aliphatic chain of from 8 to 18 carbon atoms.

8. A process of preparing a photographic polyvinyl alcohol light-sensitive silver halide emulsion as defined by claim 2, wherein said amphotolytic surface active agent is

75

a betaine having an aliphatic chain of from 8 to 18 carbon atoms.

9. A light-sensitive polyvinyl alcohol silver halide emulsion as defined by claim 1, wherein said cationic surface active agent contains an amido group as part of the molecule.

10. A process of preparing a light-sensitive photographic polyvinyl alcohol silver halide emulsion as defined by claim 2, wherein said cationic surface active agent contains an amido group as part of the molecule.

11. A light-sensitive polyvinyl alcohol silver halide emulsion as defined by claim 1, wherein said cationic surface active agent contains a sulfonamido group as part of the molecule.

12. A process of preparing a light-sensitive photographic polyvinyl alcohol silver halide emulsion as defined by claim 2, wherein said cationic surface active agent contains a sulfonamido group as part of the molecule.

13. A light-sensitive polyvinyl alcohol silver halide emulsion as defined by claim 1, wherein said amphotolytic surface active agent contains an amido group as part of the molecule.

14. A process of preparing a light-sensitive photographic polyvinyl alcohol silver halide emulsion as defined by claim 2, wherein said amphotolytic surface active agent contains an amido group as part of the molecule.

15. A light-sensitive polyvinyl alcohol silver halide emulsion as defined by claim 1, wherein said amphotolytic surface active agent contains a sulfonamido group as part of the molecule.

16. A process of preparing a light-sensitive photographic polyvinyl alcohol silver halide emulsion as defined by claim 2, wherein said amphotolytic surface active agent contains a sulfonamido group as part of the molecule.

17. A light-sensitive polyvinyl alcohol silver halide emulsion as defined by claim 1, wherein said cationic surface active agent has the following structure:



wherein X is an anion.

18. A light-sensitive polyvinyl alcohol silver halide emulsion as defined by claim 1, wherein said cationic surface active agent has the following structure:



wherein X is an anion.

19. A light-sensitive polyvinyl alcohol silver halide emulsion as defined by claim 1, wherein said cationic surface active agent has the following structure:



wherein X is an anion.

20. A process of preparing a polyvinyl alcohol silver halide emulsion as defined by claim 2, wherein said cationic surface active agent has the following structure:



wherein X is an anion.

21. A process of preparing a polyvinyl alcohol silver

halide emulsion as defined by claim 2, wherein said cationic surface active agent has the following structure:



wherein X is an anion.

22. A process of preparing a polyvinyl alcohol silver halide emulsion as defined by claim 2, wherein said cationic surface active agent has the following structure:



wherein X is an anion.

23. A light-sensitive polyvinyl alcohol silver halide emulsion as defined by claim 1, wherein said amphotolytic surface active agent has the following structure:



24. A light-sensitive polyvinyl alcohol silver halide emulsion as defined by claim 1, wherein said amphotolytic surface active agent has the following structure:



25. A process of preparing a light-sensitive polyvinyl alcohol silver halide emulsion as defined by claim 2, wherein said amphotolytic surface active agent has the following structure:



26. A process of preparing a light-sensitive polyvinyl alcohol silver halide emulsion as defined by claim 2, wherein said amphotolytic surface active agent has the following structure:



27. A process of preparing a photographic polyvinyl alcohol silver halide emulsion as defined by claim 2, wherein said ripening step is carried out in the presence of a chemical sensitizer selected from the group consisting of sodium thiosulfate, sodium tetrathionate, thiourea and thiourea derivatives.

28. A process of preparing a photographic polyvinyl alcohol silver halide emulsion as defined by claim 2, wherein said ripening step is carried out in the presence of a stabilizer capable of preventing fog in said emulsion.

#### References Cited in the file of this patent

#### UNITED STATES PATENTS

- 60 2,197,809 McQueen \_\_\_\_\_ Apr. 23, 1940  
 2,518,698 Lowe et al. \_\_\_\_\_ Aug. 15, 1950  
 2,579,016 Schupp \_\_\_\_\_ Dec. 18, 1951  
 2,624,674 Rarkington et al. \_\_\_\_\_ Jan. 6, 1953  
 2,757,089 Moessen \_\_\_\_\_ Jan. 31, 1956  
 2,848,330 Chechak et al. \_\_\_\_\_ Aug. 19, 1958  
 2,886,437 Piper \_\_\_\_\_ May 12, 1959  
 3,046,135 Beavers \_\_\_\_\_ July 24, 1962

#### FOREIGN PATENTS

- 70 116,214 Australia \_\_\_\_\_ Dec. 10, 1942  
 556,458 Great Britain \_\_\_\_\_ Oct. 6, 1942  
 558,710 Great Britain \_\_\_\_\_ Jan. 18, 1944